



US008142982B2

(12) **United States Patent**  
**Oya et al.**

(10) **Patent No.:** **US 8,142,982 B2**  
(45) **Date of Patent:** **Mar. 27, 2012**

(54) **LITHOGRAPHIC PRINTING PLATE PRECURSOR**

(75) Inventors: **Toyohisa Oya**, Shizuoka (JP); **Ryuki Kakino**, Shizuoka (JP); **Tomoya Sasaki**, Shizuoka (JP); **Yu Iwai**, Shizuoka (JP)

(73) Assignee: **Fujifilm Corporation**, Tokyo (JP)

(\*) Notice: Subject to any disclaimer, the term of this patent is extended or adjusted under 35 U.S.C. 154(b) by 298 days.

(21) Appl. No.: **12/259,885**

(22) Filed: **Oct. 28, 2008**

(65) **Prior Publication Data**

US 2009/0111049 A1 Apr. 30, 2009

(30) **Foreign Application Priority Data**

Oct. 29, 2007 (JP) ..... P2007-280310  
Oct. 29, 2007 (JP) ..... P2007-280311  
Dec. 3, 2007 (JP) ..... P2007-312315  
Dec. 3, 2007 (JP) ..... P2007-312612  
Aug. 27, 2008 (JP) ..... P2008-218847

(51) **Int. Cl.**

*G03F 7/00* (2006.01)  
*B41C 1/055* (2006.01)

(52) **U.S. Cl.** ..... **430/281.1**; 430/271.1; 430/302; 430/270.1; 101/463.1

(58) **Field of Classification Search** ..... None  
See application file for complete search history.

(56) **References Cited**

U.S. PATENT DOCUMENTS

4,640,886 A 2/1987 Miller et al.  
6,030,750 A 2/2000 Vermeersch et al.  
2001/0018159 A1 8/2001 Maemoto  
2002/0177074 A1 11/2002 Hoshi et al.  
2007/0056457 A1 \* 3/2007 Iwai et al. ..... 101/453

FOREIGN PATENT DOCUMENTS

|    |             |    |           |
|----|-------------|----|-----------|
| EP | 1 629 977   | A2 | 3/2006    |
| EP | 1 629 977   | A3 | 4/2006    |
| EP | 1 742 109   | A2 | 1/2007    |
| EP | 1754597     | A2 | 2/2007    |
| EP | 1754597     | A3 | 7/2007    |
| EP | 1 742 109   | A3 | 6/2008    |
| JP | 2938397     | B2 | 6/1999    |
| JP | 2001-277740 | A  | 10/2001   |
| JP | 2001-277742 | A  | 10/2001   |
| JP | 2002-287334 | A  | 10/2002   |
| JP | 2002-365789 | A  | * 12/2002 |

OTHER PUBLICATIONS

Derwent-2003-580576, English Abstract of Maemoto et al , Jp 2002365789 A, publication date Dec. 18, 2002, 2 pages.\*

English translation of JP, 2002-365789, A (2002) from machine translation from AIPN Japan Patent Office National Center for Industrial Property Information and Training, generated Aug. 1, 2011, 21 pages.\*

Partial European Search Report for Application No. 08018887.3 dated May 7, 2010.

European Searh Report issued in European Application No. 08 01 8887 on Dec. 22, 2010.

\* cited by examiner

*Primary Examiner* — Cynthia Hamilton

(74) **Attorney, Agent, or Firm** — Birch, Stewart, Kolasch & Birch, LLP.

(57) **ABSTRACT**

A lithographic printing plate precursor capable of being subjected to on-press development by supplying at least one of printing ink and dampening water and including a support, an image-recording layer and optionally an undercoat layer between the support and the image-recording layer, wherein at least one of the undercoat layer and the image-recording layer contains at least one of a compound represented by the formula (1A) as defined herein and a compound including a structure represented by the formula (1B) as defined herein.

**8 Claims, No Drawings**

**1**  
**LITHOGRAPHIC PRINTING PLATE  
PRECURSOR**

**FIELD OF THE INVENTION**

The present invention relates to a lithographic printing plate precursor. More particularly, it relates to a lithographic printing plate precursor capable of being subjected to image recording with laser and capable of being subjected to on-press development.

**BACKGROUND OF THE INVENTION**

In general, a lithographic printing plate is composed of an oleophilic image area accepting ink and a hydrophilic non-image area accepting dampening water in the process of printing. Lithographic printing is a printing method utilizing the nature of water and oily ink to repel with each other and comprising rendering the oleophilic image area of the lithographic printing plate to an ink-receptive area and the hydrophilic non-image area thereof to a dampening water-receptive area (ink-unreceptive area), thereby making a difference in adherence of the ink on the surface of the lithographic printing plate, depositing the ink only to the image area, and then transferring the ink to a printing material, for example, paper.

In order to produce the lithographic printing plate, a lithographic printing plate precursor (PS plate) comprising a hydrophilic support having provided thereon an oleophilic photosensitive resin layer (image-recording layer) has heretofore been broadly used. Ordinarily, the lithographic printing plate is obtained by conducting plate making according to a method of exposing the lithographic printing plate precursor through an original, for example, a lith film, and then while leaving the image-recording layer corresponding to the image area, removing the unnecessary image-recording layer corresponding to the non-image area by dissolving with an alkaline developer or a developer containing an organic solvent thereby revealing the hydrophilic surface of support.

In the hitherto known plate making process of lithographic printing plate precursor, after exposure, the step of removing the unnecessary image-recording layer by dissolving, for example, with a developer is required. However, it is one of the subjects to save or simplify such an additional wet treatment described above. Particularly, since disposal of liquid wastes discharged accompanying the wet treatment has become a great concern throughout the field of industry in view of the consideration for global environment in recent years, the demand for the solution of the above-described subject has been increased more and more.

As one of simple plate making methods in response to the above-described requirement, a method referred to as on-press development has been proposed wherein a lithographic printing plate precursor having an image-recording layer capable of being removed in the unnecessary areas during a conventional printing process is used and after exposure, the unnecessary area of the image-recording layer is removed on a printing machine to prepare a lithographic printing plate.

Specific methods of the on-press development include, for example, a method of using a lithographic printing plate precursor having an image-recording layer that can be dissolved or dispersed in dampening water, an ink solvent or an emulsion of dampening water and ink, a method of mechanically removing an image-recording layer by contact with rollers or a blanket cylinder of a printing machine, and a method of lowering cohesion of an image-recording layer or adhesion between an image-recording layer and a support upon penetration of dampening water, ink solvent or the like

**2**

and then mechanically removing the image-recording layer by contact with rollers or a blanket cylinder of a printing machine.

In the invention, unless otherwise indicated particularly, the term "development processing step" means a step of using an apparatus (ordinarily, an automatic developing machine) other than a printing machine and removing an unexposed area in an image-recording layer of a lithographic printing plate precursor upon contact with liquid (ordinarily, an alkaline developer) thereby revealing a hydrophilic surface of support. The term "on-press development" means a method or a step of removing an unexposed area in an image-recording layer of a lithographic printing plate precursor upon contact with liquid (ordinarily, printing ink and/or dampening water) by using a printing machine thereby revealing a hydrophilic surface of support.

On the other hand, digitalized technique of electronically processing, accumulating and outputting image information using a computer has been popularized in recent years, and various new image-outputting systems responding to the digitalized technique have been put into practical use. Correspondingly, attention has been drawn to a computer-to-plate technique of carrying digitalized image information on highly converging radiation, for example, a laser beam and conducting scanning exposure of a lithographic printing plate precursor with the radiation thereby directly preparing a lithographic printing plate without using a lith film. Thus, it is one of the important technical subjects to obtain a lithographic printing plate precursor adaptable to the technique described above.

In the simplification of plate making operation and the realization of dry system or non-processing system as described above, since the image-recording layer after the exposure is not fixed with the development processing, it is still sensitive to light and likely to be fogged before printing. Therefore, an image-recording layer capable of being handled in a bright room or under a yellow lamp and a light source are necessary.

As such a laser light source, a semiconductor laser emitting an infrared ray having a wavelength of 760 to 1,200 and a solid laser, for example, YAG laser, are extremely useful because these lasers having a large output and a small size are inexpensively available. Also, an UV laser can be used.

As the lithographic printing plate precursor of on-press development type capable of conducting image-recording with an infrared laser, for example, a lithographic printing plate precursor having provided on a hydrophilic support, an image-forming layer in which hydrophobic thermoplastic polymer particles are dispersed in a hydrophilic binder is described in Japanese Patent 2,938,397 (corresponding to U.S. Pat. No. 6,030,750). It is described in Japanese Patent 2,938,397 (corresponding to U.S. Pat. No. 6,030,750) that the lithographic printing plate precursor is exposed to an infrared laser to agglomerate the hydrophobic thermoplastic polymer particles by heat thereby forming an image, and mounted on a plate cylinder of a printing machine to be able to carry out on-press development by supplying dampening water and/or ink.

Although the method of forming image by the agglomeration of fine particles only upon thermal fusion shows good on-press development property, it has a problem in that the image strength is extremely weak and printing durability is insufficient.

Further, a lithographic printing plate precursor having provided on a hydrophilic support, an image-recording layer (a heat-sensitive layer) including microcapsules containing a polymerizable compound encapsulated therein is described

in JP-A-2001-277740 (the term "JP-A" as used herein means an "unexamined published Japanese patent application") and JP-A-2001-277742 (those correspond to US2001/0018159A1).

Moreover, a lithographic printing plate precursor having provided on a support an image-recording layer (a photosensitive layer) containing an imid absorbing agent, a radical polymerization initiator and a polymerizable compound is described in JP-A-2002-287334 (corresponding to US2002/0177074A1).

The methods using the polymerization reaction as described above have a feature that since the chemical bond density in the image area is high, the image strength is relatively good in comparison with the image area formed by the thermal fusion of fine polymer particles.

However, the lithographic printing plate precursor of on-press development type utilizing a polymerization reaction has a problem in that corrosion of an aluminum support is accelerated to generate dot-like (spot-like) printing stain when the image-recording layer is rendered hydrophilic to impart on-press development property. Although the generation of spot-like printing stain is prevented by rendering the image-recording layer hydrophobic, the on-press development property is degraded by the hydrophobilization of the image-recording layer. Thus, designing of the image-recording layer balancing these factors has been made but performance satisfying the both factors has not been obtained.

#### SUMMARY OF THE INVENTION

Therefore, an object of the present invention is to provide a lithographic printing plate precursor of on-press development type which is prevented from the generation of spot-like printing stain while maintaining sufficient on-press development property.

(1) A lithographic printing plate precursor capable of being subjected to on-press development by supplying at least any one of printing ink and dampening water (fountain solution) and comprising a support, an image-recording layer and optionally an undercoat layer between the support and the image-recording layer, wherein at least any one of the undercoat layer and the image-recording layer contains at least any one of a compound represented by formula (1A) shown below and a compound including a structure represented by formula (1B) shown below:



In formula (1A), R represents a substituted or unsubstituted alkyl group, a substituted or unsubstituted alkenyl group, a substituted or unsubstituted alkyne group, a substituted or unsubstituted aryl group or a substituted or unsubstituted heterocyclic group, Z represents a polyoxyethylene group or a polyoxypropylene group, Y represents a substituted or unsubstituted alkylene group having 18 or less carbon atoms, a substituted or unsubstituted arylene group having 30 or less carbon atoms or a divalent heterocyclic group, and X represents a salt of an acid group;



In formula (1B),  $\text{X}_1^+$  and  $\text{X}_2^+$ , which may be the same or different, each represents  $\text{H}^+$  or a monovalent cationic group or  $\text{X}_1^+$  and  $\text{X}_2^+$  may come together to form one divalent cationic group.

- 5 (2) The lithographic printing plate precursor as described in (1) above, wherein X in formula (1A) is a sulfonate.
- (3) The lithographic printing plate precursor as described in (1) or (2) above, wherein Z in formula (1A) is a polyoxyethylene group having a repeating unit number of 3 to 40 or a polyoxypropylene group having a repeating unit number of 3 to 40.
- 10 (4) The lithographic printing plate precursor as described in (1) above, wherein the compound including a structure represented by formula (1B) contains a polyoxyethylene group or a polyoxypropylene group in its molecule.
- 15 (5) The lithographic printing plate precursor as described in any one of (1) to (4) above, wherein the image-recording layer contains (A) an infrared absorbing agent, (B) a polymerization initiator, and (C) a polymerizable compound.
- 20 (6) The lithographic printing plate precursor as described in any one of (1) to (5) above, wherein the image-recording layer contains at least any one of a microcapsule and a microgel.
- 25 (7) The lithographic printing plate precursor as described in any one of (1) to (4) above, wherein the image-recording layer contains (A) an infrared absorbing agent and (D) a hydrophobilizing precursor.
- 30 (8) The lithographic printing plate precursor as described in any one of (1) to (7) above, which comprises a protective layer on the image-recording layer.

According to the invention, the object of the invention can be achieved by incorporating the compound having a specific structure into at least any one of the undercoat layer and the image-recording layer.

Although the function mechanism according to the invention is not quite clear, it is presumed as follows. Specifically, the reason for the generation of spot-like printing stain is that an aluminum support locally corrodes during preservation of a lithographic printing plate precursor, due to decomposition of a polymerization initiator in an image-recording layer or emission of electrons from hetero atoms in the aluminum support in neighborhood of corroded portion, dark polymerization, which is a phenomenon of polymerization of a polymerizable compound in dark, locally occurs and the portion polymerized in dark still remains on the support as a residual film after development.

It is believed that since the compound represented by formula (1A) (hereinafter, also referred simply to as a "compound (1A)") contains a polyoxyethylene group or a polyoxypropylene group and decreases the hardenability due to chain transfer property of the skeleton even when the dark polymerization occurs, the portion polymerized in dark is removable at the on-press development to prevent the generation of spot-like printing stain.

It is also believed that since the compound including a structure represented by formula (1B) (hereinafter, also referred simply to as a "compound (1B)") has the chain transfer property and decreases the hardenability, even when the dark polymerization occurs, it can be removed at the on-press development to prevent the generation of spot-like printing stain. In the case where the compound (1B) contains a polyoxyethylene group or a polyoxypropylene group, it is also believed that since the hardenability is further decreased due to the chain transfer property of the skeleton, the generation of spot-like printing stain is further prevented.

It is further believed that although the on-press development property decreases because the polyoxyethylene group

or polyoxypropylene group is insufficient in hydrophilicity, since each of the compound (1A) and compound (1B) contains a salt of acid group in the molecule thereof, a sufficient water-permeability can be obtained to achieve good on-press development property.

According to the present invention, a lithographic printing plate precursor of on-press development type which can be subjected to image recording with laser and is prevented from the generation of spot-like printing stain while maintaining sufficient on-press development property can be provided.

## DETAILED DESCRIPTION OF THE INVENTION

## [Lithographic Printing Plate Precursor]

The lithographic printing plate precursor according to the invention is capable of being subjected to on-press development by supplying at least any one of printing ink and dampening water and comprises a support, an image-recording layer and optionally an undercoat layer between the support and the image-recording layer, wherein at least any one of the undercoat layer and the image-recording layer contains at least any one of a compound represented by formula (1A) and a compound including a structure represented by formula (1B). Further, according to a preferable embodiment of the invention, the lithographic printing plate precursor has a protective layer on the image-recording layer.

(Compound Represented by Formula (1A))

The compound represented by formula (1A) is described below.



In formula (1A), R represents a substituted or unsubstituted alkyl group, a substituted or unsubstituted alkenyl group, a substituted or unsubstituted alkynyl group, a substituted or unsubstituted aryl group or a substituted or unsubstituted heterocyclic group, Z represents a polyoxyethylene group or a polyoxypropylene group, Y represents a substituted or unsubstituted alkylene group having 18 or less carbon atoms, a substituted or unsubstituted arylene group having 30 or less carbon atoms or a divalent heterocyclic group, and X represents a salt of an acid group.

Specific examples of the alkyl group represented by R include a straight-chain, branched or cyclic allyl group having from 1 to 30 carbon atoms, for example, a methyl group, an ethyl group, a propyl group, a butyl group, a pentyl group, a hexyl group, a heptyl group, an octyl group, a nonyl group, a decyl group, an isopropyl group, an isobutyl group, a sec-butyl group, a tert-butyl group, an isopentyl group, a neopen-tyl group, a 1-methylbutyl group, an isoheptyl group, a 2-ethylhexyl group, a 2-methylhexyl group, a cyclopentyl group, a cyclohexyl group, a 1-adamantyl group or a 2-norbornyl group.

Specific examples of the alkenyl group represented by R include a straight-chain, branched or cyclic alkenyl group having from 1 to 30 carbon atoms, for example, a vinyl group, a 1-propenyl group, a 1-but enyl group, a 1-methyl-1-propenyl group, a cyclopentenyl group or a cyclohexenyl group. Specific examples of the alkynyl group represented by R include an alkynyl group having from 1 to 30 carbon atoms, for example, an ethynyl group, a 1-propynyl group, a 1-butynyl group or a 1-octynyl group.

Examples of the substituent which the group represented by R may have include a monovalent non-metallic atomic group exclusive of a hydrogen atom, for example, a halogen atom (e.g., —F, —Br, —Cl or —I), a hydroxy group, an alkoxy group, an aryloxy group, a mercapto group, an alkylthio group, an arylthio group, an alkylidithio group, an

(alkyl)(OH)) and a conjugate base group thereof, an arylhydroxyboryl group (—B(aryl)(OH)) and a conjugate base group thereof, an aryl group, an alkenyl group or an alkynyl group.

Particularly, an alkoxy group, an aryloxy group, an alkoxy carbonyl group, an aryloxycarbonyl group, an N-alkylaminocarbonyl group, an N,N-dialkylaminocarbonyl group, an N-arylamino carbonyl group or an N,N-diarylamino carbonyl group is preferable.

Specific examples of the aryl group and heterocyclic group represented by R include an aryl group having from 1 to 30 carbon atoms, for example, a phenyl group, a naphthyl group or an indenyl group and a heteroaryl group having from 1 to 30 carbon atoms and containing at least one hetero atom selected from the group consisting of a nitrogen atom, an oxygen atom and a sulfur atom, for example, a furyl group, a thienyl group, a pyrrolyl group, a pyridyl group or a quinolyl group.

For R in formula (1A) according to the invention, the alkyl group is particularly preferable.

Z represents a polyoxyethylene group or a polyoxypropylene group in which a number of repeating unit is preferably from 2 to 100, more preferably from 3 to 40.

Specific examples of the alkylene group represented by Y include a straight-chain, branched or cyclic alkylene group having from 1 to 30 carbon atoms, for example, a methylene group, an ethylene group, a propylene group, a butylene group, a pentylene group, a hexylene group, a heptylene group, an octylene group, a nonylene group, a decylene group, a cyclopentylene group, a cyclohexylene group, an adamantylene group or a norbornylene group.

Specific examples of the arylene group and divalent heterocyclic group represented by Y include an arylene group having from 1 to 30 carbon atoms, for example, a phenylene group, a naphthylene group or an indenylene group and a heteroaryl group having from 1 to 30 carbon atoms and containing at least one hetero atom selected from the group consisting of a nitrogen atom, an oxygen atom and a sulfur atom, for example, a divalent group derived from furan, thiophene, pyrrolidine, pyridine or quinoline, respectively.

10 Of the groups represented by Y, the alkylene group is preferable.

The salt of an acid group represented by X is not particularly restricted as long as it is a salt of an acid group.

15 Of the salts of an acid group, salts of an acid group represented by (1) to (3) described below are preferable.

(1) a carboxylic acid group (—CO<sub>2</sub>H)

(2) a sulfonic acid group (—SO<sub>3</sub>H)

(3) a phosphoric acid group (—PO<sub>3</sub>H<sub>2</sub>)

20 Of the acid group represented by (1) to (3), (2) sulfonic acid group is preferable.

The cationic group for forming the salt with the acid group in X is not particularly restricted as long as it is a cationic group.

25 Of the cationic groups, an inorganic cationic group, for example, a lithium cation, a sodium cation or a potassium cation and an organic cationic group, for example, a quaternary ammonium group or a quaternary phosphonium group are preferable.

30 Specific examples of the compound (1A) are set forth below, but the invention should not be construed as being limited thereto.



**9****10**-continued  
A-(18)

A-(19)



A-(20)



A-(21)



A-(22)



A-(23)



A-(24)



A-(25)



A-(26)



A-(27)



A-(28)



A-(29)



A-(30)



A-(31)



A-(32)



A-(33)



A-(34)



A-(35)



A-(36)



A-(37)



A-(38)



A-(39)



A-(40)



A-(41)



A-(42)



A-(43)



A-(44)



A-(45)



## 11

(Compound Including Structure Represented by Formula (1B))

The compound including a structure represented by formula (1B) is described below.



In formula (1B),  $\text{X}_1^+$  and  $\text{X}_2^+$ , which may be the same or different, each represents  $\text{H}^+$  or a monovalent cationic group or  $\text{X}_1^+$  and  $\text{X}_2^+$  may come together to form one divalent cationic group.

Examples of the monovalent cationic group include an inorganic cationic group, for example, a lithium cation, a sodium cation or a potassium cation and an organic cationic group, for example, a quaternary ammonium group or a quaternary phosphonium group. Examples of the divalent cationic group include a cation including two organic cationic groups, for example, a quaternary ammonium group or a quaternary phosphonium group in its molecule and a divalent inorganic cation, for example, a magnesium ion or a calcium ion.

Of the cationic groups, a sodium ion is particularly preferable.

It is also preferred that the compound including a structure represented by formula (1B) contains a polyoxyethylene group or a polyoxypropylene group in its molecule. A number of repeating unit of oxyethylene unit or oxypropylene unit is preferably from 1 to 100, more preferably from 2 to 80, still more preferably from 3 to 40. By the introduction of polyoxyethylene group or polyoxypropylene group, the effect of preventing the generation of spot-like printing stain is improved. When the number of repeating unit of oxyethylene unit or oxypropylene unit is larger than 100, solubility in a coating solution is deteriorated.

Of the compounds including a structure represented by formula (1B), a compound having a stricture represented by formula (1B2) shown below is preferable.



In formula (1B2), R represents an alkyl group which may have a substituent or an aryl group which may have a substituent, n represents an integer of 0 to 20, and  $\text{X}_1^+$  and  $\text{X}_2^+$  have the same meanings as  $\text{X}_1^+$  and  $\text{X}_2^+$  in formula (1B), respectively.

The alkyl group may be any of a straight chain, branched and cyclic form and has preferably from 1 to 20 carbon atoms, more preferably from 1 to 16 carbon atoms, most preferably from 1 to 12 carbon atoms. Specific examples of the alkyl group include a methyl group, an ethyl group, a butyl group, a 2-ethylhexyl group, a cyclohexyl group, a decyl group, a dodecyl group and a hexadecyl group. Examples of the substituent for the alkyl group include a fatty acid amido group and an alkoxy group each having 20 or less carbon atoms.

## 12

Examples of the aryl group include a phenyl group, a butylphenyl group, an amylphenyl group, an octylphenyl group and a nonylphenyl group.

The compound including a stricture represented by formula (1B) may have two or more strictures represented by formula (1B). Specific examples thereof include compounds in which plural groups formed by eliminating one hydrogen atom from R in formula (1B2) are connected through a single bond or a connecting group. The connecting group is not particularly restricted and includes an alkylene group, an arylene group, a divalent or higher heterocyclic group and a trivalent or higher hydrocarbon group.

Specific examples of the compound (1B) are set forth below, but the invention should not be construed as being limited thereto.



**13**

-continued

**14**

-continued



The compound having a structure represented by formula 35 (1B) can be synthesized according to a known method described, for example, in JP-A-2002-356697.

The amount of the compound (1A) or (1B) added (total amount of the compounds (1A) and (1B) when both of them are added) to the image-recording layer is preferably from 0.5 to 20% by weight, more preferably from 1 to 10% by weight still more preferably from 2 to 8% by weight based on the total solid content of the image-recording layer.

The amount of the compound (1A) or (1B) added (total amount of the compounds (1A) and (1B) when both of them are added) to the undercoat layer is preferably from 1 to 100% by weight, more preferably from 5 to 95% by weight, still more preferably from 10 to 90% by weight, based on the total solid content of the undercoat layer.

The compound (1A) or (1B) may be incorporated into both the undercoat layer and the image-recording layer.

In the range described above, a lithographic printing plate precursor having good on-press development property and prevented from the generation of spot-like printing stain is obtained. The compounds (1A) and (1B) may be used individually or as a mixture of two or more thereof. Specifically, two or more compounds selected from either the compound (1A) or the compound (1B) may be used or two or more compounds selected from both the compound (1A) and the compound (1B) may be used.

B-(19) 60 (Image-Recording Layer)

The image-recording layer for use in the invention is an image-recording layer capable of forming an image by supplying printing ink and dampening water on a printing machine after image exposure to remove the unexposed area.

The representative image-forming mechanism enabling the on-press development included in the image-recording layer includes (1) an embodiment wherein (A) an infrared absorb-

15

ing agent, (B) a polymerization initiator and (C) a polymerizable compound are included and an image area is hardened utilizing the polymerization reaction and (2) an embodiment wherein (A) an infrared absorbing agent and (D) a hydrophobilizing precursor are included and a hydrophobic region (image area) is formed utilizing heat fusion or heat reaction of the hydrophobilizing precursor. A mixture of these two embodiments may also used. For instance, the hydrophobilizing precursor (D) may be incorporated into the image-recording layer of polymerization type (1) or the polymerizable compound and the like may be incorporated into the image-recording layer of hydrophobilizing precursor type (2). Among them, the embodiment of polymerization type including the infrared absorbing agent (A), polymerization initiator (B) and polymerizable compound (C) is preferable.

The image-forming element and component of the image-recording layer other than the compounds (1A) and (1B) will be described in greater detail below.

<(A) Infrared Absorbing Agent>

In the case wherein the lithographic printing plate precursor according to the invention is subjected to the image formation using as a light source, a laser emitting an infrared ray of 760 to 1,200 nm, it is ordinarily essential to use an infrared absorbing agent. The infrared absorbing agent has a function of converting the infrared ray absorbed to heat and a function of being excited by the infrared ray to perform electron transfer/energy transfer to a polymerization initiator (radical generator) described hereinafter. The infrared absorbing agent for use in the invention includes a dye and pigment each having an absorption maximum in a wavelength range of 760 to 1,200 nm.

As the dye, commercially available dyes and known dyes described in literatures, for example, *Senryo Binran* (Dye Handbook) compiled by The Society of Synthetic Organic

16

Chemistry, Japan (1970) can be used. Specifically, the dyes includes azo dyes, metal complex azo dyes, pyrazolone azo dyes, naphthoquinone dyes, anthraquinone dyes, phthalocyanine dyes, carbonium dyes, quinoneimine dyes, methine dyes, cyanine dyes, squarylium dyes, pyrylium salts and metal thiolate complexes.

Examples of preferable dye include cyanine dyes described, for example, in JP-A-58-125246, JP-A-59-84356 and JP-A-60-78787, methine dyes described, for example, in JP-A-58-173696, JP-A-58-181690 and JP-A-58-194595, 10 naphthoquinone dyes described, for example, in JP-A-58-112793, JP-A-58-224793, JP-A-59-48187, JP-A-59-73996, JP-A-60-52940 and JP-A-60-63744, squarylium dyes described, for example, in JP-A-58-112792, and cyanine dyes described, for example, in British Patent 434,875.

15 Also, near infrared absorbing sensitizers described in U.S. Pat. No. 5,156,938 are preferably used. Further, substituted arylbenzo(thio)pyrylium salts described in U.S. Pat. No. 3,881,924, trimethinethiopyrylium salts described in JP-A-57-142645 (corresponding to U.S. Pat. No. 4,327,169), pyrylium compounds described in JP-A-58-181051, JP-A-58-220143, JP-A-5-941363, JP-A-59-84248, JP-A-59-84249, JP-A-59-146063 and JP-A-59-146061, cyanine dyes described in JP-A-59-216146, pentamethinethiopyrylium salts described in U.S. Pat. No. 4,283,475, and pyrylium compounds described in JP-B-5-13514 (the term "JP-B" as used herein means an "examined Japanese patent publication") and JP-B-5-19702 are also preferably used. Other preferable examples of the dye include near infrared absorbing dyes represented by formulae (I) and (II) in U.S. Pat. No. 4,756,993.

20 Other preferable examples of the infrared absorbing dye according to the invention include specific indolenine cyanine dyes described in JP-A-2002-278057 as illustrated below.





Of the dyes, cyanine dyes, squarylium dyes, pyrylium dyes, nickel thiolate complexes and indolenine cyanine dyes are preferred. Further, cyanine dyes and indolenine cyanine dyes are more preferred. As a particularly preferable example of the dye, a cyanine dye represented by formula (i) shown below is exemplified.

Formula (i):



In formula (i),  $X^1$  represents a hydrogen atom, a halogen atom,  $-\text{NPh}_2$ ,  $X^2-\text{L}^1$  or a group represented by the structural formula shown below.  $X^2$  represents an oxygen atom, a nitrogen atom or a sulfur atom,  $\text{L}^1$  represents a hydrocarbon group having from 1 to 12 carbon atoms, an aromatic ring containing a hetero atom or a hydrocarbon group having from 1 to 12 carbon atoms and containing a hetero atom. The hetero atom used herein indicates a nitrogen atom, a sulfur atom, an oxygen atom, a halogen atom or a selenium atom.  $R^a$  represents a substituent selected from a hydrogen atom, an alkyl group, an aryl group, a substituted or unsubstituted amino group and a halogen atom, and  $X_a^-$  has the same meaning as  $Z_a^-$  defined hereinafter.



$R^1$  and  $R^2$  each independently represents a hydrocarbon group having from 1 to 12 carbon atoms. In view of the preservation stability of a coating solution for image-recording layer, it is preferred that  $R^1$  and  $R^2$  each represents a hydrocarbon group having two or more carbon atoms, and it is particularly preferred that  $R^1$  and  $R^2$  are combined with each other to form a 5-membered or 6-membered ring.

$\text{Ar}^1$  and  $\text{Ar}^2$ , which may be the same or different, each represents an aromatic hydrocarbon group which may have a substituent. Preferable examples of the aromatic hydrocarbon group include a benzene ring and a naphthalene ring. Also, preferable examples of the substituent include a hydrocarbon group having 12 or less carbon atoms, a halogen atom and an alkoxy group having 12 or less carbon atoms, and a hydrocarbon group having 12 or less carbon atoms and an alkoxy group having 12 or less carbon atoms are most preferable.  $Y^1$

-continued

and  $Y^2$ , which may be the same or different, each represents a sulfur atom or a dialkylmethylen group having 12 or less carbon atoms.  $R^3$  and  $R^4$ , which may be the same or different, each represents a hydrocarbon group having 20 or less carbon atoms, which may have a substituent. Preferable examples of the substituent include an alkoxy group having 12 or less carbon atoms, a carboxyl group and a sulfo group, and an alkoxy group having 12 or less carbon atoms is most preferable.  $R^5$ ,  $R^6$ ,  $R^7$  and  $R^8$ , which may be the same or different, each represents a hydrogen atom or a hydrocarbon group having 12 or less carbon atoms. In view of the availability of raw materials, a hydrogen atom is preferred.  $Za^1$  represents a counter anion. However,  $Za^-$  is not necessary when the cyanine dye represented by formula (i) has an anionic substituent in the structure thereof and neutralization of charge is not needed. Preferable examples of the counter ion for  $Za^-$  include a halogen ion, a perchlorate ion, a tetrafluoroborate ion, a hexafluorophosphate ion and a sulfonate ion, and particularly preferable examples thereof include a perchlorate ion, a tetrafluoroborate ion, a hexafluorophosphate ion and an arylsulfonate ion in view of the preservation stability of a coating solution for image-recording layer.

Specific examples of the cyanine dye represented by formula (i), which can be preferably used in the invention, include those described in paragraph Nos. [0017] to [0019] of JP-A-2001-133969.

Further, other particularly preferable examples include specific indolenine cyanine dyes described in JP-A-2002-278057 described above.

Examples of the pigment for use in the invention include commercially available pigments and pigments described in Colour Index (C.I.), *Saisin Ganryo Binran* (Handbook of the Newest Pigments) compiled by Pigment Technology Society of Japan (1977), *Saishin Ganryo Oyou Gijutsu* (Newest Application on Technologies for Pigments), CMC Publishing Co., Ltd. (1986) and *Insatsu Ink Gijutsu* (Printing Ink Technology), CMC Publishing Co., Ltd. (1984).

Examples of the pigment include black pigments, yellow pigments, orange pigments, brown pigments, red pigments, purple pigments, blue pigments, green pigments, fluorescent pigments, metal powder pigments and polymer-bonded dyes.

Specific examples of usable pigment include insoluble azo pigments, azo lake pigments, condensed azo pigments, chelated azo pigments, phthalocyanine pigments, anthraquinone pigments, perylene and perynone pigments, thioindigo pigments, quinacridone pigments, dioxazine pigments, isoindolinone pigments, quinophthalone pigments, dying lake pigments, azine pigments, nitroso pigments, nitro pigments, natural pigments, fluorescent pigments, inorganic pigments and carbon black. Of the pigments, carbon black is preferred.

The pigment may be used without undergoing surface treatment or may be used after the surface treatment. For the surface treatment, a method of coating a resin or wax on the surface, a method of attaching a surfactant and a method of

bonding a reactive substance (for example, a silane coupling agent, an epoxy compound or polyisocyanate) to the pigment surface. The surface treatment methods are described in *Kinzoku Seiken no Seishitsu to Oyo* (Properties and Applications of Metal Soap), Sawai Shobo, *Insatsu Ink Gijutsu* (Printing Ink Technology), CMC Publishing Co., Ltd. (1984), and *Saishin Ganryo Oyo Gijutsu* (Newest Application on Technologies for Pigments), CMC Publishing Co., Ltd. (1986).

The pigment has a particle size of preferably from 0.01 to 10  $\mu\text{m}$ , more preferably from 0.05 to 1  $\mu\text{m}$ , particularly preferably from 0.1 to 1  $\mu\text{m}$ . In the range described above, good stability of the pigment dispersion in the coating solution for image-recording layer and good uniformity of the image-recording layer can be obtained.

For dispersing the pigment, a known dispersion technique for use in the production of ink or toner may be used. Examples of the dispersing machine include an ultrasonic dispersing machine, a sand mill, an attritor, a pearl mill, a super-mill, a ball mill, an impeller, a disperser, a KD mill, a colloid mill, a dynatron, a three roll mill and a pressure kneader. The dispersing machines are described in detail in *Saishin Ganryo Oyo Gijutsu* (Newest Application on Technologies for Pigments), CMC Publishing Co., Ltd. (1986).

The infrared absorbing agent may be added together with other components to the same image-recording layer or may be added to a different image-recording layer separately provided. With respect to the amount of the infrared absorbing agent added, in the case of preparing a negative-working lithographic printing plate precursor, the amount is so controlled that absorbance of the image-recording layer at the maximum absorption wavelength in the wavelength region of 760 to 1,200 nm measured by reflection measurement is in a range of 0.3 to 1.2, preferably in a range of 0.4 to 1.1. In the range described above the polymerization reaction proceeds uniformly in the thickness direction of the image-recording layer and good film strength of the image area and good adhesion property of the image area to the support are achieved.

The absorbance of the image-recording layer can be controlled depending on the amount of the infrared absorbing agent added to the image-recording layer and the thickness of the image-recording layer. The measurement of the absorbance can be carried out in a conventional manner. The method for measurement includes, for example, a method of forming an image-recording layer having a thickness determined appropriately in the range necessary for the lithographic printing plate precursor on a reflective support, for example, an aluminum plate, and measuring reflection density of the image-recording layer by an optical densitometer or a spectrophotometer according to a reflection method using an integrating sphere.

<(B) Polymerization Initiator>

The polymerization initiator (B) for use in the invention is a compound that generates a radical with light energy, heat energy or both energies to initiate or accelerate polymerization of polymerizable compound (C). The polymerization initiator for use in the invention includes, for example, known thermal polymerization initiators, compounds containing a bond having small bond dissociation energy and photopolymerization initiators.

The polymerization initiators in the invention include, for example, (a) organic halides, (b) carbonyl compounds, (c) azo compounds, (d) organic peroxides, (e) metallocene compounds, (f) azido compounds, (g) hexaarylbimidazole compounds, (h) organic borate compounds, (i) disulfone compounds, (j) oxime ester compounds and (k) onium salt compounds.

The organic halides (a) described above specifically include, for example, compounds described in Wakabayashi et al., *Bull. Chem. Soc. Japan*, 42, 2924 (1969), U.S. Pat. No. 3,905,815, JP-B-46-4605, JP-A-48-35281, JP-A-55-32070, 5 JP-A-60-239736, JP-A-61-169835, JP-A-61-169837, JP-A-62-58241, JP-A-62-212401, JP-A-63-70243, JP-A-63-298339 and M. P. Huff, *Journal of Heterocyclic Chemistry*, 1, No. 3 (1970). Particularly, oxazole compounds and s-triazine compounds each substituted with a trihalomethyl group are 10 preferably exemplified.

More preferably, s-triazine derivatives and oxadiazole derivatives each of which has at least one of mono-, di- and tri-halogen substituted methyl groups connected are exemplified. Specific examples thereof include 2,4,6-tris(monochloromethyl)-s-triazine, 2,4,6-tris(trichloromethyl)-s-triazine, 2-methyl-4,6-bis(trichloromethyl)-s-triazine, 2-n-propyl-4,6-bis(trichloromethyl)-s-triazine, 2-( $\alpha$ , $\alpha$ , $\beta$ -trichloroethyl)-4,6-bis(trichloromethyl)-s-triazine, 2-phenyl-4,6-bis(trichloromethyl)-s-triazine, 2-p-methoxyphenyl)-4,6-bis(trichloromethyl)-s-triazine, 2-(3,4-epoxyphenyl)-4,6-bis(trichloromethyl)-s-triazine, 2-(p-chlorophenyl)-4,6-bis(trichloromethyl)-s-triazine, 2-(p-bromophenyl)-4,6-bis(trichloromethyl)-s-triazine, 2-(p-fluoroxyphenyl)-4,6-bis(trichloromethyl)-s-triazine, 2-(p-trifluoromethylphenyl)-4,6-bis(trichloromethyl)-s-triazine; 2-(2,6-dichlorophenyl)-4,6-bis(trichloromethyl)-s-triazine, 2-(2,6-difluorophenyl)-4,6-bis(trichloromethyl)-s-triazine, 2-(2,6-dibromophenyl)-4,6-bis(trichloromethyl)-s-triazine, 2-(4-biphenyl)-4,6-bis(trichloromethyl)-s-triazine, 2-(4'-chloro-4-biphenyl)-4,6-bis(trichloromethyl)-s-triazine, 2-(p-cyanophenyl)-4,6-bis(trichloromethyl)-s-triazine, 2-(p-acetylphenyl)-4,6-bis(trichloromethyl)-s-triazine, 2-(p-ethoxycarbonylphenyl)-4,6-bis(trichloromethyl)-s-triazine, 2-(p-phenoxy carbonylphenyl)-4,6-bis(trichloromethyl)-s-triazine, 2-(p-methylsulfonylphenyl)-4,6-bis(trichloromethyl)-s-triazine, 2-(p-dimethylsulfoniumphenyl)-4,6-bis(trichloromethyl)-s-triazine tetrafluoroborate, 2-(2,4-difluorophenyl)-4,6-bis(trichloromethyl)-s-triazine, 2-(p-diethoxyphosphorylphenyl)-4,6-bis(trichloromethyl)-s-triazine, 2-[4-(4-hydroxyphenylcarbonylamino)phenyl]-4,6-bis(trichloromethyl)-s-triazine, 2-[4-(p-methoxyphenyl)-1,3-butadienyl]-4,6-bis(trichloromethyl)-s-triazine, 2-(p-methoxystyryl)-4,6-bis(trichloromethyl)-s-triazine, 2-(p-isopropoxy styryl)-4,6-bis(trichloromethyl)-s-triazine, 2-(p-tolyl)-4,6-bis(trichloromethyl)-s-triazine, 2-(4-methoxynaphthyl)-4,6-bis(trichloromethyl)-s-triazine, 2-phenylthio-4,6-bis(trichloromethyl)-s-triazine, 2-benzylthio-4,6-bis(trichloromethyl)-s-triazine, 2,4,6-tris(dibromomethyl)-s-triazine, 2,4,6-tris(tribromomethyl)-s-triazine, 2-methyl-4,6-bis(tribromomethyl)-s-triazine, 2-methoxy-4,6-bis(tribromomethyl)-s-triazine, 2-(o-methoxystyryl)-5-trichloromethyl-1,3,4-oxadiazole, 2-(3,4-epoxystyryl)-5-trichloromethyl-1,3,4-oxadiazole, 2-[1-phenyl-2-(4-methoxyphenyl)vinyl]-5-trichloromethyl-1,3,4-oxadiazole, 2-(p-hydroxystyryl)-5-trichloromethyl-1,3,4-oxadiazole, 2-(3,4-dihydroxystyryl)-5-trichloromethyl-1,3,4-oxadiazole and 60 2-(p-tert-butoxystyryl)-5-trichloromethyl-1,3,4-oxadiazole.

The carbonyl compounds (b) include, for example, benzophenone derivatives, e.g., benzophenone, Michler's ketone, 2-methylbenzophenone, 3-methylbenzophenone, 4-methylbenzophenone, 2-chlorobenzophenone, 4-bromobenzophenone or 2-carboxybenzophenone, acetophenone derivatives, e.g., 2,2-dimethoxy-2-phenylacetophenone, 2,2-

## 21

diethoxyacetophenone, 1-hydroxycyclohexylphenylketone,  $\alpha$ -hydroxy-2-methylphenylpropanone, 1-hydroxy-1-methyl-ethyl-(p-isopropylphenyl)ketone, 1-hydroxy-1-(p-dodecylphenyl)ketone, 2-methyl-(4'-methylthio)phenyl-2-morpholino-1-propanone or 1,1,1-trichloromethyl-(p-butylphenyl)ketone, thioxantone derivatives, e.g., thioxantone, 2-ethylthioxantone, 2-isopropylthioxantone, 2-chlorothioxantone, 2,4-dimethylthioxantone, 2,4-diethylthioxantone or 2,4-diisopropylthioxantone, and benzoic acid ester derivatives, e.g., ethyl p-dimethylaminobenzoate or ethyl p-diethylaminobenzoate.

The azo compounds (c) include, for example, azo compounds described in JP-A-8-108621.

The organic peroxides (d) include, for example, trimethyl-cyclohexanone peroxide, acetylacetone peroxide, 1,1-bis (tert-butylperoxy)-3,3,5-trimethylcyclohexane, 1,1-bis(tert-butylperoxy)cyclohexane, 2,2-bis(tert-butylperoxy)butane, tert-butylhydroperoxide, cumene hydroperoxide, diisopropylbenzene hydroperoxide, 2,5-dimethylhexane-2,5-dihydroperoxide, 1,1,3,3-tetramethylbutyl hydroperoxide, tert-butylcumyl peroxide, dicumyl peroxide, 2,5-dimethyl-2,5-di(tert-butylperoxy)hexane, 2,5-oxanoyl peroxide, succinic peroxide, benzoyl peroxide, 2,4-dichlorobenzoyl peroxide, diisopropylperoxy dicarbonate, di-2-ethylhexylperoxy dicarbonate, di-2-ethoxyethylperoxy dicarbonate, dimethoxyisopropylperoxy dicarbonate, di(3-methyl-3-methoxybutyl)peroxy dicarbonate, tert-butylperoxy acetate, tert-butylperoxy pivalate, tert-butylperoxy neodecanoate, tert-butylperoxy octanoate, tert-butylperoxy laurate, tersyl carbonate, 3,3',4,4'-tetra(tert-butylperoxycarbonyl)benzophenone, 3,3',4,4'-tetra(tert-hexylperoxycarbonyl)benzophenone, 3,3',4,4'-tetra(p-isopropylcumylperoxycarbonyl)benzophenone, carbonyl di(tert-butylperoxydihydrogen diphthalate) and carbonyl di(tert-hexylperoxydihydrogen diphthalate).

The metallocene compounds (e) include, for example, various titanocene compounds described in JP-A-59-152396, JP-A-61-151197, JP-A-63-41484, JP-A-2-249, JP-A-2-4705 and JP-A-5-83588, for example, dicyclopentadienyl-Ti-bisphenyl, dicyclopentadienyl-Ti-bis-2,6-difluorophen-1-yl, dicyclopentadienyl-Ti-bis-2,4-difluorophen-1-yl, dicyclopentadienyl-Ti-bis-2,4,6-trifluorophen-1-yl, dicyclopentadienyl-Ti-bis-2,3,5,6-tetrafluorophen-1-yl, dicyclopentadienyl-Ti-bis-2,3,4,5,6-pentafluorophen-1-yl, dimethylcyclopentadienyl-Ti-bis-2,6-difluorophen-1-yl, dimethylcyclopentadienyl-Ti-bis-2,4,6-trifluorophen-1-yl, dimethylcyclopentadienyl-Ti-bis-2,3,5,6-tetrafluorophen-1-yl, dimethylcyclopentadienyl-Ti-bis-2,3,4,5,6-pentafluorophen-1-yl or dicyclopentadienyl-Ti-bis-2,6-difluoro-3-(pyrol-1-yl)phen-1-yl, and iron-arene complexes described in JP-A-1-304453 and JP-A-1-152109.

The azido compounds (f) include, for example, 2,6bis(4-azidobenzylidene)-4-methylcyclohexanone.

The hexaarylbiiimidazole compounds (g) include, for example, various compounds described in JP-B-6-29285 and U.S. Pat. Nos. 3,479,185, 4,311,783 and 4,622,286, specifically, for example, 2,2'-bis(o-chlorophenyl)-4,4',5,5'-tetraphenylbiiimidazole, 2,2'-bis(o-bromophenyl)-4,4',5,5'-tetraphenylbiiimidazole, 2,2'-bis(o,p-dichlorophenyl)-4,4',5,5'-tetraphenylbiiimidazole, 2,2'-bis(o-chlorophenyl)-4,4',5,5'-tetrakis(m-methoxyphenyl)biiimidazole, 2,2'-bis(o,o'-dichlorophenyl)-4,4',5,5'-tetraphenylbiiimidazole, 2,2'-bis(o-nitrophenyl)-4,4',5,5'-tetraphenylbiiimidazole, 2,2'-bis(o-methylphenyl)-4,4',5,5'-tetraphenylbiiimidazole or 2,2'-bis(o-trifluoromethylphenyl)-4,4',5,5'-tetraphenylbiiimidazole.

The organic borate compounds (h) include, for example, organic borates described in JP-A-62-143044, JP-A-62-150242, JP-A-9-188685, JP-A-9-188686, JP-A-9-188710,

## 22

JP-A-2000-131837, JP-A-2002-107916, Japanese Patent 2,764,769, JP-A-2002-116539 and Martin Kunz, *Rad Tech '98, Proceeding*, Apr. 19-22 (1998), Chicago, organic boron sulfonium complexes or organic boron oxosulfonium complexes described in JP-A-6-157623, JP-A-6-175564 and JP-A-6-175561, organic boron iodonium complexes described in JP-A-6-175554 and JP-A-6-175553, organic boron phosphonium complexes described in JP-A-9-188710, and organic boron transition metal coordination complexes described in JP-A-6-348011, JP-A-7-128785, JP-A-7-140589, JP-A-7-306527 and JP-A-7-292014.

The disulfone compounds (i) include, for example, compounds described in JP-A-61-166544 and JP-A-2002-328465.

The oxime ester compounds (j) include, for example, compounds described in *J. C. S. Perkin II*, 1653-1660 (1979), *J. C. S. Perkin II*, 156-162 (1979), *Journal of Photopolymer Science and Technology*, 202-232 (1995) and JP-A-2000-66385, and compounds described in JP-A-2000-80068. Specific examples thereof include compounds represented by the following structural formulae:



**23**

-continued

**24**

-continued





25 The onium salt compounds (k) include, for example, diazonium salts described in S. I. Schlesinger, *Photogr. Sci. Eng.*, 18,387 (1974) and T. S. Bat et al., *Polymer*, 21, 423 (1980), ammonium salts described in U.S. Pat. No. 4,069,055 and JP-A-4-365049, phosphonium salts described in U.S. Pat. 30 Nos. 4,069,055 and 4,069,056, iodonium salts described in European Patent 104,143, U.S. Pat. Nos. 339,049 and 410, 201, JP-A-2-150848 and JP-A-2-296514, sulfonium salts described in European Patents 370,693, 390,214, 233,567, 297,443 and 297,442, U.S. Pat. Nos. 4,933,377, 161,811, 410,201, 339,049, 4,760,013, 4,734,444 and 2,833,827 and German Patents 2,904,626, 3,604,580 and 3,604,581, seleniumium salts described in J. V. Crivello et al., *Macromolecules*, 10 (6), 1307 (1977) and J. V. Crivello et al., *J. Polymer Sci., Polymer Chem. Ed.*, 17, 1047 (1979), and arsonium salts 35 described in C. S. Wen et al., *Teh. Proc. Conf. Rad. Curing ASIA*, p. 478, Tokyo, October (1988).

Particularly, in view of reactivity and stability, the oxime ester compounds and diazonium salts, iodonium salts and sulfonium salts described above are preferably exemplified.  
 45 In the invention, the onium salt functions not as an acid generator but as an ionic radical polymerization initiator.

The onium salts preferably used in the invention include onium salts represented by the following formulae (RI-I) to (RI-III):



In formula (RI-I),  $\text{Ar}^{11}$  represents an aryl group having 20 or less carbon atoms, which may have 1 to 6 substituents. Preferable example of the substituent includes an alkyl group having from 1 to 12 carbon atoms, an alkenyl group having

from 1 to 12 carbon atoms, an alkynyl group having from 1 to 12 carbon atoms, an aryl group having from 1 to 12 carbon atoms, an alkoxy group having from 1 to 12 carbon atoms an aryloxy group having from 1 to 12 carbon atoms, a halogen atom, an alkylamino group having from 1 to 12 carbon atoms, a dialkylamino group having from 1 to 12 carbon atoms, an alkylamido group or arylamido group having from 1 to 12 carbon atoms, a carbonyl group, a carboxyl group, a cyano group, a sulfonyl group, an thioalkyl group having from 1 to 12 carbon atoms and an thioaryl group having from 1 to 12 carbon atoms.  $Z^{11-}$  represents a monovalent anion and specifically includes a halogen ion, a perchlorate ion, a hexafluorophosphate ion, a tetrafluoroborate ion, a sulfonate ion, a sulfinate ion, a thosulfonate ion and a sulfate ions. From the standpoint of stability and visibility of print-out image, a perchlorate ion, a hexafluorophosphate ion, a tetrafluoroborate ion, a sulfonate ion or a sulfinate ion is preferable.

In the formula (RI-II),  $Ar^{21}$  and  $Ar^{22}$  each independently represents an aryl group having 20 or less carbon atoms, which may have 1 to 6 substituents. Preferable example of the substituent includes an alkyl group having from 1 to 12 carbon atoms, an alkenyl group having from 1 to 12 carbon atoms, an alkynyl group having from 1 to 12 carbon atoms, an aryl group having from 1 to 12 carbon atoms, an alkoxy group having from 1 to 12 carbon atoms, an aryloxy group having from 1 to 12 carbon atoms, a halogen atom, an alkylamino group having from 1 to 12 carbon atoms, a dialkylamino group having from 1 to 12 carbon atoms, an alkylamido group or arylamido group having from 1 to 12 carbon atoms, a carbonyl group, a carboxyl group, a cyano group, a sulfonyl group, an thioalkyl group having from 1 to 12 carbon atoms and an thioaryl group having from 1 to 12 carbon atoms.  $Z^{21-}$  represents a monovalent anion and specifically includes a halogen ion, a perchlorate ion, a hexafluorophosphate ion, a tetrafluoroborate ion, a sulfonate ion, a sulfinate ion, a thosulfonate ion, a sulfate ion and a carboxylate ion. From the standpoint of stability and visibility of print-out image, a perchlorate ion, a hexafluorophosphate ion, a tetrafluoroborate ion, a sulfonate ion, a sulfinate ion or a carboxylate ion is preferable.

In the formula (RI-III),  $R^{31}$ ,  $R^{32}$  and  $R^{33}$  each independently represents an aryl group having 20 or less carbon atoms, which may have 1 to 6 substituents, an alkyl group, an alkenyl group or an alkynyl group and is preferably an aryl group from the standpoint of reactivity and stability. Preferable example of the substituent includes an alkyl group having from 1 to 12 carbon atoms, an alkenyl group having from 1 to 12 carbon atoms, an alkynyl group having from 1 to 12 carbon atoms, an aryl group having from 1 to 12 carbon atoms, an alkoxy group having from 1 to 12 carbon atoms, an aryloxy group having from 1 to 12 carbon atoms, a halogen atom, an alkylamino group having from 1 to 12 carbon atoms, a dialkylamino group having from 1 to 12 carbon atoms, an alkylamido group or arylamido group having from 1 to 12 carbon atoms, a carbonyl group, a carboxyl group, a cyano group, a sulfonyl group, an thioalkyl group having from 1 to 12 carbon atoms and an thioaryl group having from 1 to 12 carbon atoms.  $Z^{31-}$  represents a monovalent anion and specifically includes a halogen ion, a perchlorate ion, a hexafluorophosphate ion, a tetrafluoroborate ion, a sulfonate ion, a sulfinate ion, a thosulfonate ion, a sulfate ion and a carboxylate ion. From the standpoint of stability and visibility of print-out image, a perchlorate ion, a hexafluorophosphate ion, a tetrafluoroborate ion, a sulfonate ion, a sulfinate ion or a carboxylate ion is preferable. Carboxylate ions described in JP-A-2001-343742 are more preferable, and carboxylate ions described in JP-A-2002-148790 are particularly preferable.

Specific examples of the onium salt compound preferably used as the polymerization initiator in the invention are set forth below, but the invention should not be construed as being limited thereto.



(N-2)



(N-3)



(N-4)

(N-5)

(N-6)



(N-7)

(N-8)



(N-9)

(N-10)



**29**

-continued

PF<sub>6</sub><sup>-</sup>ClO<sub>4</sub><sup>-</sup>PF<sub>6</sub><sup>-</sup>**30**

-continued

(I-4)

ClO<sub>4</sub><sup>-</sup>

(N-11)

10

(N-12)

15

(N-13)

20

CF<sub>3</sub>SO<sub>3</sub><sup>-</sup>

(I-7)

(I-8)

(I-9)



(I-10)



(I-11)



(I-12)



(I-1)

50

(N-17)

45

(I-2)

55

(I-3)

60

(I-4)

65

(I-5)



(I-15)

**31**  
-continued

(I-16)



5

ClO4^-

(I-17)

PF6^-

(I-18)

C4F9SO3^-

(I-19)



25



30

CF3COO^-

(I-21)

CF3SO3^-

(I-22)



(I-24)

45



50

(I-25)



(I-26)

60



65

C4F9COO^-**32**  
-continued

(I-27)



(I-28)



(I-29)



(I-30)



(I-31)

PF6^-C4F9SO3^-

(I-32)



(I-33)



(I-34)



(I-35)



(I-36)

PF6^-

**33**  
-continued

C4F9SO3^-PF6^-ClO4^-CF3SO3^-COO^-

(I-37)

5

(I-38)

(I-39) 15

(S-1)

(S-2)

(S-3) 35

(S-4)

(S-5) 45

(S-6)

(S-7)

(S-8)

(S-9)

65

**34**  
-continued

(S-10)



(S-11)

(S-12)

(S-13)

(S-14)

(S-15)

(S-16)

(S-17)

35

-continued

(S-18)



36

and esters or amides thereof. Preferably, esters of an unsaturated carboxylic acid with an aliphatic polyhydric alcohol compound and amides of an unsaturated carboxylic acid with an aliphatic polyvalent amine compound are used. An addition reaction product of an unsaturated carboxylic acid ester or amide having a nucleophilic substituent for example, a hydroxy group, an amino group or a mercapto group, with a monofunctional or polyfunctional isocyanate or epoxy, or a dehydration condensation reaction product of the unsaturated

- 10 carboxylic acid ester or amide with a monofunctional or polyfunctional carboxylic acid is also preferably used. Furthermore, an addition reaction product of an unsaturated carboxylic acid ester or amide having an electrophilic substituent, for example, an isocyanato group or an epoxy group with a monofunctional or polyfunctional alcohol, amine or thiol, or a substitution reaction product of an unsaturated carboxylic acid ester or amide having a releasable substituent, for example, a halogen atom or a tosyloxy group with a monofunctional or polyfunctional alcohol, amine or thiol is also 15 preferably used. In addition, compounds in which the unsaturated carboxylic acid described above is replaced by an unsaturated phosphonic acid, styrene, vinyl ether or the like 20 can also be used.

With respect to specific examples of the monomer, which is

- 25 an ester of an aliphatic polyhydric alcohol compound with an unsaturated carboxylic acid, an acrylic acid ester includes, for example, ethylene glycol diacrylate, triethylene glycol diacrylate, 1,3-butanediol diacrylate, tetramethylene glycol diacrylate, propylene glycol diacrylate, neopentyl glycol diacrylate, trimethylolpropane triacrylate, trimethylolpropane tri (acryloyloxypropyl)ether, trimethylolethane triacrylate, hexanediol diacrylate, 1,4-cyclohexanediol diacrylate, tetraethylene glycol diacrylate, pentaerythritol diacrylate, pentaerythritol triacrylate, pentaerythritol tetraacrylate, dipentaerythritol diacrylate, dipentaerythritol hexaacrylate, sorbitol triacrylate, sorbitol tetraacrylate, sorbitol pentaacrylate, sorbitol hexaacrylate, tri(acryloyloxyethyl) isocyanurate, polyester acrylate oligomer and isocyanuric acid EO modified triacrylate.

- 30 40 A methacrylic acid ester includes, for example, tetramethylene glycol dimethacrylate, triethylene glycol dimethacrylate, neopentyl glycol dimethacrylate, trimethylolpropane trimethacrylate, trimethylolethane trimethacrylate, ethylene glycol dimethacrylate, 1,3-butanediol dimethacrylate, hexanediol dimethacrylate, pentaerythritol dimethacrylate, pentaerythritol trimethacrylate, pentaerythritol tetramethacrylate, dipentaerythritol dimethacrylate, dipentaerythritol hexamethacrylate, sorbitol trimethacrylate, sorbitol tetramethacrylate, bis[p-(3-methacryloxy-2-hydroxypropoxy) phenyl]dimethylmethane and bis[p-(methacryloxyethoxy) phenyl]dimethylmethane.

- 35 45 50 An itaconic acid ester includes, for example, ethylene glycol diitaconate, propylene glycol diitaconate, 1,3-butanediol diitaconate, 1,4-butanediol diitaconate, tetramethylene glycol diitaconate, pentaerythritol diitaconate and sorbitol tetraitaconate.

- 55 60 A crotonic acid ester includes, for example, ethylene glycol dicrotonate, tetramethylene glycol dicrotonate, pentaerythritol dicrotonate and sorbitol tetracrotonate.

- An isocrotonic acid ester includes, for example, ethylene glycol diisocrotonate, pentaerythritol diisocrotonate and sorbitol tetraisocrotonate.

- A maleic acid ester includes, for example, ethylene glycol dimaleate, triethylene glycol dimaleate, pentaerythritol dimaleate and sorbitol tetramaleate.

- 65 Other examples of the ester, which can be preferably used, include aliphatic alcohol esters described in JP-B-51-47334

The polymerization initiator (B) is not limited to those described above. In particular, the organic halides (a), particularly the triazine type initiators included therein, the oxime ester compounds (j), the diazonium salts, iodonium salts and sulfonium salts included in the onium salt compounds (k) are more preferable from the standpoint of reactivity and stability. Of the polymerization initiators, onium salt compounds including as a counter ion, an inorganic anion, for example,  $\text{PF}_6^-$  or  $\text{BF}_4^-$  are preferable in combination with the infrared absorbing agent from the standpoint of improvement in the visibility of print-out image. Further, in view of excellence in the color-forming property, a diaryliodonium is preferable as the onium salt.

Further, the polymerization initiator (B) may be added together with other components to the same layer or may be added to an image-recording layer or a different layer provided adjacent thereto.

The polymerization initiator can be added preferably in an amount from 0.1 to 50% by weight, more preferably from 0.5 to 30% by weight particularly preferably from 0.8 to 20% by weight, based on the total solid content of the image-recording layer in the range described above, good sensitivity and good stain resistance in the non-image area at the time of printing are obtained. The polymerization initiators may be used individually or in combination of two or more thereof.

<(C) Polymerizable Compound>

The polymerizable compound (C) for use in the invention is an addition-polymerizable compound having at least one ethylenically unsaturated double bond, and it is selected from compounds having at least one, preferably two or more, terminal ethylenically unsaturated double bonds. Such compounds are widely known in the field of art and they can be used in the invention without any particular limitation. The compound has a chemical form, for example, a monomer, a prepolymer, specifically, a dimer, a trimer or an oligomer, or a copolymer thereof, or a mixture thereof. Examples of the monomer and copolymer thereof include unsaturated carboxylic acids (for example, acrylic acid, methacrylic acid, itaconic acid, crotonic acid, isocrotonic acid or maleic acid)

and JP-A-57-196231, esters having an aromatic skeleton described in JP-A-59-5240, JP-A-59-5241 and JP-A-2-226149, and esters containing an amino group described in JP-A-1-165613.

The above-described ester monomers can also be used as a mixture.

Specific examples of the monomer, which is an amide of an aliphatic polyvalent amine compound with an unsaturated carboxylic acid, include methylene bisacrylamide, methylene bismethacrylamide, 1,6-hexamethylene bisacrylamide, 1,6-hexamethylene bismethacrylamide, diethylenetriamine trisacrylamide, xylylene bisacrylamide and xylylene bis-methacrylamide. Other preferable examples of the amide monomer include amides having a cyclohexylene structure described in JP-B-54-21726.

Urethane type addition polymerizable compounds produced using an addition reaction between an isocyanate and a hydroxy group are also preferably used, and specific examples thereof include vinylurethane compounds having two or more polymerizable vinyl groups per molecule obtained by adding a vinyl monomer containing a hydroxy group represented by formula (A) shown below to a polyisocyanate compound having two or more isocyanate groups per molecule, described in JP-B-48-41708.



wherein  $\text{R}^4$  and  $\text{R}^5$  each independently represents H or  $\text{CH}_3$ .

Also, urethane acrylates described in JP-A-51-37193, JP-B-2-32293 and JP-B-2-16765, and urethane compounds having an ethylene oxide skeleton described in JP-B-58-49860, JP-B-56-17654, JP-B-62-39417 and JP-B-62-39418 are preferably used. Furthermore, a photopolymerizable composition having remarkably excellent photosensitive speed can be obtained by using an addition polymerizable compound having an amino structure or a sulfide structure in its molecule, described in JP-A-63-277653, JP-A-63-260909 and JP-A-1-105238.

Other examples include polyfunctional acrylates and methacrylates, for example, polyester acrylates and epoxy acrylates obtained by reacting an epoxy resin with acrylic acid or methacrylic acid, described in JP-A-48-64183, JP-B-49-43191 and JP-B-52-30490. Specific unsaturated compounds described in JP-B-46-43946, JP-B-1-40337 and JP-B-1-40336, and vinylphosphonic acid type compounds described in JP-A-2-25493 can also be exemplified. In some cases, structure containing a perfluoroalkyl group described in JP-A-61-22048 can be preferably used. Moreover, photo-curable monomers or oligomers described in *Nippon Sekachaku Kyokaishi (Journal of Japan Adhesion Society)*, Vol. 20, No. 7, pages 300 to 308 (1984) can also be used.

Details of the method of using the polymerizable compound, for example, selection of the structure, individual or combination use, or an amount added, can be appropriately arranged depending on the characteristic design of the final lithographic printing plate precursor. For instance, the compound is selected from the following standpoints.

In view of the sensitivity, a structure having a large content of unsaturated groups per molecule is preferred and in many cases, a bifunctional or more functional compound is preferred. In order to increase the strength of image area, that is, cured layer, a trifunctional or more functional compound is preferred. A combination use of compounds different in the functional number or in the kind of polymerizable group (for example, an acrylic acid ester, a methacrylic acid ester, a styrene compound or a vinyl ether compound) is an effective method for controlling both the sensitivity and the strength.

The selection and use method of the polymerizable compound are also important factors for the compatibility and dispersibility with other components (for example, a binder polymer, a polymerization initiator or a coloring agent) in the image-recording layer. For instance, the compatibility may be improved in some cases by using the compound of low purity or using two or more kinds of the compounds in combination. A specific structure may be selected for the purpose of improving an adhesion property to a support or a protective layer described hereinafter. The polymerizable compound is preferably used in an amount from 5 to 80% by weight, more preferably from 25 to 75% by weight, based on the nonvolatile component of the image-recording layer. The polyineritable compounds may be used individually or in combination of two or more thereof.

In the method of using the polymerizable compound, the structure blend and amount added can be appropriately selected by taking account of the extent of polymerization inhibition due to oxygen, resolution, fogging property, change in refractive index, surface tackiness and the like. Further, depending on the case, a layer construction, for example, an undercoat layer or an overcoat layer, and a coating method, may also be considered.

<(D) Hydrophobilizing Precursor>

The hydrophobilizing precursor for use in the invention is a fine particle capable of converting the image-recording layer to be hydrophobic when heat is applied. The fine particle is preferably at least one fine particle selected from hydrophobic thermoplastic polymer fine particles and thermo-reactive polymer fine particles.

As the hydrophobic thermoplastic polymer fine particles for use in the image-recording layer, hydrophobic thermoplastic polymer fine particles described, for example, in *Research Disclosure*, No. 33303, January (1992), JP-A-9-123387, JP-A-9-131850, JP-A-9-171249, JP-A-9-171250 and European Patent 931,647 are preferably exemplified. Specific examples of the polymer constituting the polymer fine particle include a homopolymer or copolymer of a monomer, for example, ethylene, styrene, vinyl chloride, methyl acrylate, ethyl acrylate, methyl methacrylate, ethyl methacrylate, vinylidene chloride, acrylonitrile or vinyl carbazole, and a mixture thereof. Of the polymers, polystyrene and polymethyl methacrylate are more preferable.

The average particle size of the hydrophobic thermoplastic polymer fine particle for use in the invention is preferably from 0.01 to 2.0  $\mu\text{m}$ .

Synthesis methods of the hydrophobic thermoplastic polymer fine particle having the particle size described above which can be used as the hydrophobilizing precursor include an emulsion polymerization method and a suspension polymerization method and in addition, a method (dissolution dispersion method) of dissolving the above compound in a water-insoluble organic solvent, mixing and emulsifying the solution with an aqueous solution containing a dispersant and applying heat to the emulsion thereby solidifying the emulsion to a fine particle state while volatilizing the organic solvent.

The thermo-reactive polymer fine particle which can be used as the hydrophobilizing precursor in the invention includes a thermosetting polymer fine particle and a polymer fine particle having a thermo-reactive group and they form a hydrophobilized region by crosslinkage due to thermal reaction and change in the functional group involved therein.

As the thermosetting polymer, a resin having a phenolic skeleton, a urea resin (for example, a resin obtained by resinification of urea or a urea derivative, for example, methoxymethylated urea, with an aldehyde, for example, formalde-

hyde), a melamine resin (for example, a resin obtained by resinification of melamine or a melamine derivative with an aldehyde, for example, formaldehyde), an alkyd resin, an unsaturated polyester resin, a polyurethane resin and an epoxy resin are exemplified. Of the resins, a resin having a phenolic skeleton, a melamine resin, a urea resin and an epoxy resin are especially preferable.

Preferable examples of the resin having a phenolic skeleton include a phenolic resin obtained by resinification of phenol or cresol with an aldehyde, for example, formaldehyde, a hydroxystyrene resin and a polymer or copolymer of methacrylamide, acrylamide, methacrylate or acrylate having a phenolic skeleton, for example, N-(p-hydroxyphenyl)methacrylamide or p-hydroxyphenyl methacrylate.

The average particle size of the thermosetting polymer fine particle for use in the invention is preferably from 0.01 to 2.0  $\mu\text{m}$ . While the thermosetting polymer fine particle can be easily obtained by a dissolution dispersion method, a thermosetting polymer may be made fine particle when the thermosetting polymer is synthesized. However, the invention should not be construed as being limited to these methods.

As the thermo-reactive group of the polymer fine particle having a thermo-reactive group for use in the invention, a functional group performing any reaction can be used as long as a chemical bond is formed. For instance, an ethylenically unsaturated group (for example, an acryloyl group, a methacryloyl group, a vinyl group or an allyl group), a cationic polymerizable group (for example, a vinyl group or a vinyloxy group) performing a radical polymerization reaction, an isocyanate group performing an addition reaction or a blocked form thereof an epoxy group, a vinyloxy group and a functional group having an active hydrogen atom (for example, an amino group, a hydroxy group or a carboxyl group) of the reaction partner, a carboxyl group performing a condensation reaction and a hydroxyl group or an amino group of the reaction partner, and an acid anhydride performing a ring opening addition reaction and an amino group or a hydroxyl group of the reaction partner are preferably exemplified.

The introduction of the functional group into polymer fine particle may be conducted at the polymerization or by utilizing a polymer reaction after the polymerization.

When the functional group is introduced at the polymerization, it is preferred that the monomer having the functional group is subjected to emulsion polymerization or suspension polymerization. Specific examples of the monomer having the functional group include allyl methacrylate, allyl acrylate, vinyl methacrylate, vinyl acrylate, 2-(vinyloxy)ethyl methacrylate, p-vinyloxystyrene, p-[2-(vinyloxy)ethyl]styrene, glycidyl methacrylate, glycidyl acrylate, 2-isocyanatoethyl methacrylate or a blocked isocyanato thereof, for example, with an alcohol, 2-isocyanatoethyl acrylate or a blocked isocyanato thereof, for example, with an alcohol, 2-aminoethyl methacrylate, 2-aminoethyl acrylate, 2-hydroxyethyl methacrylate, 2-hydroxyethyl acrylate, acrylic acid, methacrylic acid, maleic anhydride, a difunctional acrylate and a difunctional methacrylate, but the invention should not be construed as being limited to thereto.

In the invention, a copolymer of the monomer having the functional group and a monomer having no thermo-reactive group copolymerizable with the monomer can also be used. Examples of the copolymerizable monomer having no thermo-reactive group include styrene, an alkyl acrylate, an alkyl methacrylate, acrylonitrile and vinyl acetate, but the copolymerizable monomer having no thermo-reactive group should not be construed as being limited thereto.

As the polymer reaction used in the case where the thermo-reactive group is introduced after the polymerization, polymer reactions described, for example, in WO 96/34316 can be exemplified.

- 5 Of the polymer fine particles having a thermo-reactive group, polymer fine particles which are coalesced with each other by heat are preferable, and those having a hydrophilic surface and dispersible in water are particularly preferable. It is preferred that the contact angle (water droplet in air) of a
- 10 film prepared by coating only the polymer fine particle and drying the particle at temperature lower than the solidification temperature is lower than the contact angle (water droplet in a) of a film prepared by coating only the polymer fine particle and drying at temperature higher than the solidification temperature.
- 15 For making the surface of polymer fine particle hydrophilic, it is effective to let a hydrophilic polymer or oligomer, for example, polyvinyl alcohol or polyethylene glycol, or a hydrophilic low molecular weight compound adsorb on the surface of the polymer fine particle. However,
- 20 the method for hydrophilizing the surface of polymer fine particle should not be construed as being limited hereto.

The solidification temperature of the polymer fine particle having a thermo-reactive group is preferably 70°C. or higher, more preferably 100°C. or higher in consideration of the time-lapse stability. The average particle size of the polymer fine particle is preferably from 0.01 to 2.0  $\mu\text{m}$ , more preferably from 0.05 to 2.0  $\mu\text{m}$ , particularly preferably from 0.1 to 1.0  $\mu\text{m}$ . In the range described above, good resolution and good time-lapse stability can be achieved.

30 <Microcapsule and/or Microgel>

In the invention, several embodiments can be employed in order to incorporate the above-described constituting components (A) to (C) of the image-recording layer and other constituting components described hereinafter into the image-recording layer. One embodiment is an image-recording layer of molecular dispersion type prepared by dissolving the constituting components in an appropriate solvent to coat as described, for example, in JP-A-2002-287334. Another embodiment is all image-recording layer of microcapsule type prepared by encapsulating all or part of the constituting components into microcapsules to incorporate into the image-recording layer as described, for example, in JP-A-2001-277740 and JP-A-2001-277742. In the image-recording layer of microcapsule type, the constituting components may be present outside the microcapsules. It is a more preferable embodiment of the image-recording layer of microcapsule type that hydrophobic constituting components are encapsulated in microcapsules and hydrophilic components are present outside the microcapsules.

45 50 A still another embodiment is an image-recording layer containing a crosslinked resin particle, that is, a microgel. The microgel can contain a part of the constituting components (A) to (C) inside and/or on the surface thereof. Particularly, an embodiment of a reactive microgel containing the polymerizable compound (C) on the surface thereof is preferable in view of the image-forming sensitivity and printing durability.

55 In order to achieve more preferable on-press development property, the image-recording layer is preferably the image-recording layer of microcapsule type or microgel type.

60 65 As a method of microencapsulation or microgelation of the constituting components of the image-recording layer, known methods can be used.

Methods of producing the microcapsule include, for example, a method of utilizing coacervation described in U.S. Pat. Nos. 2,800,457 and 2,800,458, a method of using interfacial polymerization described in U.S. Pat. No. 3,287,154, JP-B-38-19574 and JP-B-42-446, a method of using deposi-

tion of polymer described in U.S. Pat. Nos. 3,418,250 and 3,660,304, a method of using an isocyanate polyol wall material described in U.S. Pat. No. 3,796,669, a method of using an isocyanate wall material described in U.S. Pat. No. 3,914,511, a method of using a urea-formaldehyde-type or urea-formaldehyde-resorcinol-type wall-forming material described in U.S. Pat. Nos. 4,001,140, 4,087,376 and 4,089,802, a method of using a wall material, for example, a melamine-formaldehyde resin or hydroxycellulose described in U.S. Pat. No. 4,025,445, an in-situ method by monomer polymerization described in JP-B-36-9163 and JP-B-51-9079, a spray drying method described in British Patent 93 0,422 and U.S. Pat. No. 3,111,407, and an electrolytic dispersion cooling method described in British Patents 952,807 and 967,074, but the invention should not be construed as being limited thereto.

A preferable microcapsule wall used in the invention has three-dimensional crosslinking and has a solvent-swellable property. From this point of view, a preferable wall material of the microcapsule includes polyurea, polyurethane, polyester, polycarbonate, polyamide and a mixture thereof, and polyurea and polyurethane are particularly preferred. Further, a compound having a crosslinkable functional group, for example, an ethylenically unsaturated bond, capable of being introduced into the binder polymer described hereinafter may be introduced into the microcapsule wall.

On the other hand, methods of preparing the microgel include, for example, a method of utilizing granulation by interfacial polymerization described in JP-B-38-19574 and JP-B-42-446 and a method of utilizing granulation by dispersion polymerization in a non-aqueous system described in JP-A-5-61214, but the invention should not be construed as being limited thereto.

To the method utilizing interfacial polymerization, known production methods of microcapsule can be applied.

The microgel preferably used in the invention is granulated by interfacial polymerization and has three-dimensional crosslinking. From this point of view, a preferable material to be used includes polyurea, polyurethane, polyester, polycarbonate, polyamide and a mixture thereof, and polyurea and polyurethane are particularly preferred.

The average particle size of the microcapsule or microgel is preferably from 0.01 to 3.0  $\mu\text{m}$ , more preferably from 0.05 to 2.0  $\mu\text{m}$ , particularly preferably from 0.10 to 1.0  $\mu\text{m}$ . In the range described above, good resolution and good time-lapse stability can be achieved.

#### <Other Components of Image-Recording Layer>

The image-recording layer according to the invention may further contain various additives, if desired. Such additives will be described below.

#### <1> Binder Polymer

In the image-recording layer according to the invention, a binder polymer can be used for the purpose of improving a film strength of the image-recording layer. The binder polymer which can be used in the invention can be selected from those heretofore known without restriction and polymers having a film-forming property are preferable. Examples of the binder polymer include acrylic resins, polyvinyl acetal resins, polyurethane resins, polyurea resins, polyimide resins, polyamide resins, epoxy resins, methacrylic resins, polystyrene resins, novolac type phenolic resins, polyester resins, synthesis rubbers and natural rubbers.

The binder polymer may have a crosslinkable property in order to improve the film strength of the image area. In order to impart the crosslinkable property to the binder polymer, a crosslinkable functional group, for example, an ethylenically unsaturated bond is introduced into a main chain or side chain

of the polymer. The crosslinkable functional group may be introduced by copolymerization.

Examples of the polymer having an ethylenically unsaturated bond in the main chain thereof include poly-1,4-butadiene and poly-1,4-isoprene.

Examples of the polymer having an ethylenically unsaturated bond in the side chain thereof include a polymer of an ester or amide of acrylic acid or methacrylic acid, which is a polymer wherein the ester or amide residue (R in  $-\text{COOR}$  or  $-\text{CONHR}$ ) has an ethylenically unsaturated bond.

Examples of the residue (R described above) having an ethylenically unsaturated bond include  $-(\text{CH}_2)_n\text{CR}^1=\text{CR}^2\text{R}^3$ ,  $-(\text{CH}_2\text{O})_n\text{CH}_2\text{CR}^1=\text{CR}^2\text{R}^3$ ,  $-(\text{CH}_2\text{CH}_2\text{O})_n\text{CH}_2\text{CR}^1=\text{CR}^2\text{R}^3$ ,  $-(\text{CH}_2)_n\text{NH}-\text{CO}-\text{O}-\text{CH}_2\text{CR}^1=\text{CR}^2\text{R}^3$ ,  $-(\text{CH}_2)_n-\text{O}-\text{CO}-\text{CR}^1=\text{CR}^2\text{R}^3$  and  $-(\text{CH}_2\text{CH}_2\text{O})_2-\text{X}$  (wherein R<sup>1</sup> to R<sup>3</sup> each represents a hydrogen atom, a halogen atom or an alkyl group having from 1 to 20 carbon atoms, an aryl group, alkoxy group or aryloxy group, or R<sup>1</sup> and R<sup>2</sup> or R<sup>1</sup> and R<sup>3</sup> may be combined with each other to form a ring. n represents an integer of 1 to 10. X represents a dicyclopentadienyl residue).

Specific examples of the ester residue include  $-\text{CH}_2\text{CH}=\text{CH}_2$  (described in JP-B-7-21633),  $-\text{CH}_2\text{CH}_2\text{O}-\text{CH}_2\text{CH}=\text{CH}_2$ ,  $-\text{CH}_2\text{C}(\text{CH}_3)=\text{CH}_2$ ,  $-\text{CH}_2\text{CH}=\text{CH}-\text{C}_6\text{H}_5$ ,  $-\text{CH}_2\text{CH}_2\text{OCOCH}=\text{CH}-\text{C}_6\text{H}_5$ ,  $-\text{CH}_2\text{CH}_2-\text{NHCOO}-\text{CH}_2\text{CH}=\text{CH}_2$  and  $-\text{CH}_2\text{CH}_2\text{O}-\text{X}$  (wherein X represents a dicyclopentadienyl residue).

Specific examples of the amide residue include  $-\text{CH}_2\text{CH}=\text{CH}_2$ ,  $-\text{CH}_2\text{CH}_2-\text{Y}$  (wherein Y represents a cyclohexene residue) and  $-\text{CH}_2\text{CH}_2-\text{OCO}-\text{CH}=\text{CH}_2$ .

The binder polymer having crosslinkable property is cured, for example, by addition of a free radical (a polymerization initiating radical or a growing radical of a polymerizable compound during polymerization) to the crosslinkable functional group of the polymer and undergoing addition polymerization between the polymers directly or through a polymerization chain of the polymerizable compound to form crosslinkage between the polymer molecules. Alternately, it is cured by generation of a polymer radical upon extraction of an atom (for example, a hydrogen atom on a carbon atom adjacent to the functional crosslinkable group) in the polymer by a free radical and connecting the polymer radicals with each other to form cross-linkage between the polymer molecules.

The content of the crosslinkable group in the binder polymer (content of the radical polymerizable unsaturated double bond determined by iodine titration) is preferably from 0.1 to 10.0 mmol, more preferably from 1.0 to 7.0 mmol, most preferably from 2.0 to 5.5 mmol, based on 1 g of the binder polymer. In the range described above, good sensitivity and good preservation stability can be obtained.

From the standpoint of improvement in the on-press development property in the unexposed area of the image-recording layer, it is preferred that the binder polymer has high solubility or high dispersibility in ink and/or dampening water. In order to increase the solubility or dispersibility in the ink, the binder polymer is preferably oleophilic and in order to increase the solubility or dispersibility in the dampening water, the binder polymer is preferably hydrophilic. Therefore, it is effective in the invention that an oleophilic binder polymer and a hydrophilic binder polymer are used in combination.

The hydrophilic binder polymer preferably includes, for example, a polymer having a hydrophilic group, for example, a hydroxy group, a carboxyl group, a carboxylate group, a hydroxyethyl group, a polyoxyethyl group, a hydroxypropyl group, a polyoxypropyl group, an amino group, an aminoet-

hyl group, an aminopropyl group, an ammonium group, an amido group, a carboxymethyl group, a sulfonic acid group or a phosphoric acid group.

Specific examples the hydrophilic binder polymer include gum arabic, casein, gelatin, a starch derivative, carboxy methyl cellulose and a sodium salt thereof, cellulose acetate, sodium alginate, a vinyl acetate-maleic acid copolymer, a styrene-maleic acid copolymer, polyacrylic acid and a salt thereof, polymethacrylic acid and a salt thereof, a homopolymer or copolymer of hydroxyethyl methacrylate, a homopolymer or copolymer of hydroxyethyl acrylate, a homopolymer or copolymer of hydroxypropyl methacrylate, a homopolymer or copolymer of hydroxypropyl acrylate, a homopolymer or copolymer of hydroxybutyl methacrylate, a homopolymer or copolymer of hydroxybutyl acrylate, a polyethylene glycol, a hydroxypropylene polymer, polyvinyl alcohol, a hydrolyzed polyvinyl acetate having a hydrolysis degree of 60% by mole or more, preferably 80% by mole or more, polyvinyl formal, polyvinyl butyral, polyvinyl pyrrolidone, a homopolymer or copolymer of acrylamide, a homopolymer or polymer of methacrylamide, a homopolymer or copolymer of N-methylolacrylamide, polyvinyl pyrrolidone, an alcohol-soluble nylon, a polyether of 2,2-bis-(4-hydroxyphenyl)propane and epichlorohydrin.

The weight average molecular weight (Mw) of die binder polymer is preferably 5,000 or more, more preferably from 10,000 to 300,000. The number average molecular weight (Mn) of the binder polymer is preferably 1,000 or more, more preferably from 2,000 to 250,000. The polydispersity (Mw/Mn) thereof is preferably from 1.1 to 10.

The binder polymer is available by purchasing a commercial product or synthesizing according to a known method.

The content of the binder polymer is ordinarily from 5 to 90% by weight, preferably from 5 to 80% by weight, more preferably from 10 to 70% by weight based on the total solid content of the image-recording layer. In the range described above, good strength of the image area and good image-forming property can be obtained.

It is preferred that the polymerizable compound (C) and the binder polymer are used in a weight ratio of 0.5/1 to 4/1.

<2> Surfactant

In the image-recording layer according to the invention, a surfactant can be used in order to promote the on-press development property and to improve the state of coated surface. The surfactant used includes, for example, a nonionic surfactant, an anionic surfactant, a cationic surfactant, an amphoteric surfactant and a fluorine-based surfactant. The surfactants may be used individually or in combination of two or more thereof.

The nonionic surfactant used in the invention is not particular restricted, and those hitherto known can be used. Examples of the nonionic surfactant include polyoxyethylene alkyl ethers, polyoxyethylene alkyl phenyl ethers, polyoxyethylene polystyryl phenyl ethers, polyoxyethylene polyoxypropylene alkyl ethers, glycerin fatty acid partial esters, sorbitan fatty acid partial esters, pentaerythritol fatty acid partial esters, propylene glycol monofatty acid esters, sucrose fatty acid partial esters, polyoxyethylene sorbitan fatty acid partial esters, polyoxyethylene sorbitol fatty acid partial esters, polyethylene glycol fatty acid esters, polyglycerol fatty acid partial esters, polyoxyethylenated castor oils, polyoxyethylene glycerol fatty acid partial esters, fatty acid diethanolamides, N,N-bis-2-hydroxyalkylamines, polyoxyethylene alkylamines, triethanolamine fatty acid esters, trialkylamine oxides, polyethylene glycols, and copolymers of polyethylene glycol and polypropylene glycol.

The anionic surfactant used in the invention is not particularly restricted and those hitherto known can be used. Examples of the anionic surfactant include fatty acid salts, abietic acid salts, hydroxyalkanesulfonic acid salts, alkane-sulfonic acid salts, dialkylsulfosuccinic ester salts, straight-chain alkylbenzenesulfonic acid salts, branched alkylbenzenesulfonate acid salts, alkylnaphthalenesulfonic acid salts, alkylphenoxypolyoxyethylene propylsulfonic acid salts, polyoxyethylene alkylsulfophenyl ether salts, N-methyl-N-oleyltaurine sodium salt, N-alkylsulfosuccinic monoamide disodium salts, petroleum sulfonic acid salts, sulfated beef tallow oil, sulfate ester salts of fatty acid alkyl ester, alkyl sulfate ester salts, polyoxyethylene all ether sulfate ester salts, fatty acid monoglyceride sulfate ester salts, polyoxyethylene alkyl phenyl ether sulfate ester salts, polyoxyethylene styrylphenyl ether sulfate ester salts, alkyl phosphate ester salts, polyoxyethylene alkyl ether phosphate ester salts, partial saponification products of styrene/maleic anhydride copolymer, partial saponification products of olefin/maleic anhydride copolymer and naphthalene sulfonate formalin condensates.

The cationic surfactant used in the invention is not particularly restricted and those hitherto known can be used. Examples of the cationic surfactant include alkylamine salts, quaternary ammonium salts, polyoxyethylene alkyl amine salts and polyoxyethylene polyamine derivatives.

The amphoteric surfactant used in the invention is not particularly restricted and those hitherto known can be used. Examples of the amphoteric surfactant include carboxybetaines, aminocarboxylic acids, sulfobetaines, aminosulfic esters, and imidazolines.

In the surfactants described above, the term "polyoxyethylene" can be replaced with "polyoxyalkylene", for example, polyoxymethylene, polyoxypropylene or polyoxybutylene, and such surfactants can also be used in the invention.

Further, a preferable surfactant includes a fluorine-based surfactant containing a perfluoroalkyl group in its molecule. Examples of the fluorine-based surfactant include an anionic type, for example, perfluoroalkyl carboxylates, perfluoroalkyl sulfonates or perfluoroalkyl phosphates; an amphoteric type, for example, perfluoroalkyl betaines; a cationic type, for example, perfluoroalkyl trimethyl ammonium salts; and a nonionic type, for example, perfluoroalkyl amine oxides, perfluoroalkyl ethylene oxide adducts, oligomers having a perfluoroalkyl group and a hydrophilic group, oligomers having a perfluoroalkyl group and an oleophilic group, oligomers having a perfluoroalkyl group, a hydrophilic group and an oleophilic group or urethanes having a perfluoroalkyl group and an oleophilic group. Further, fluorine-based surfactants described in JP-A-62-170950, JP-A-62-226143 and JP-A-60-168144 are also preferably exemplified.

The surfactants can be used individually or in combination of two or more thereof.

The content of the surfactant is preferably from 0.001 to 10% by weight, more preferably from 0.01 to 5% by weight, based on the total solid content of the image-recording layer.

<3> Coloring Agent

In the image-recording layer according to the invention, a dye having a large absorption in the visible region can be used as a coloring agent of the image formed. Specifically, the dye includes Oil yellow #101, Oil yellow #103, Oil pink #312, Oil green BG, Oil blue BOS, Oil blue #603, Oil black BY, Oil black BS, Oil black T-505 (produced by Orient Chemical Industries, Ltd.), Victoria pure blue, Crystal violet (CI42555), Methyl violet (CI42535), Ethyl violet, Rhodamine B (CI45170B), Malachite green (CI42000), Methylene blue

(CI52015) and dyes described in JP-A-62-293247. Further, a pigment, for example, a phthalocyanine pigment, an azo pigment, carbon black or titanium oxide can also preferably be used.

It is preferred to add the coloring agent since distinction between the image area and the non-image area is easily conducted after the formation of image. The amount of the coloring agent added is preferably from 0.01 to 10% by weight based on the total solid content of the image-recording layer.

<4> Print-Out Agent

To the image-recording layer according to the invention, a compound undergoing discoloration with an acid or radical can be added in order to form a printout image. As a compound used for such a purpose, various dyes, for example, of diphenylmethane type, triphenylmethane type, thiazine type, oxazine type, xanthene type, anthraquinone type, iminoquinone type, azo type and azomethine type are effectively used.

Specific examples thereof include dyes, for example, Brilliant green, Ethyl violet, Methyl green, Crystal violet, basic Fuchsin, Methyl violet 2B, Quinaldine red, Rose Bengal, Methanyl yellow, Thimol sulfophthalein, Xylenol blue, Methyl orange, Paramethyl red, Congo red, Benzo purpurin 4B,  $\alpha$ -Naphthyl red, Nile blue 2B, Nile blue A, Methyl violet, Malachite green, Parafuchsin, Victoria pure blue BOH (produced by Hodogaya Chemical Co., Ltd.), Oil blue #603 (produced by Orient Chemical Industries, Ltd.), Oil pink #312 produced by Orient Chemical Industries, Ltd.), Oil red 5B produced by Orient Chemical Industries, Ltd.), Oil scarlet #308 (produced by Orient Chemical Industries, Ltd.), Oil red OG (produced by Orient Chemical Industries, Ltd.), Oil red RR (produced by Orient Chemical Industries, Ltd.), Oil green #502 (produced by Orient Chemical Industries, Ltd.), Spiron Red BEH special (produced by Hodogaya Chemical Co., Ltd.), m-Cresol purple, Cresol red, Rhodamine B, Rhodamine 6G, Sulfo rhodamine B, Auramine, 4-p-diethylaminophenyliminonaphthoquinone, 2-carboxyanilino-4-p-diethylaminophenyliminonaphthoquinone, 2-carboxystearylamino-4-p-N,N-bis(hydroxyethyl)aminophenyliminonaphthoquinone, 1-phenyl-3-methyl-4-p-diethylaminophenylimino-5-pyrazolon or 1- $\beta$ -naphthyl-4-p-diethylaminophenylimino-5-pyrazolon, and a leuco dye, for example, p, p', p"-hexamethyltriaminotriphenylmethane (leuco crystal violet) or Pergascript Blue SRB (produced by Ciba Geigy Ltd.).

In addition to those described above, a leuco dye known as a material for heat-sensitive paper or pressure-sensitive paper is also preferably used. Specific examples thereof include crystal violet lactone, malachite green lactone, benzoyl leuco methylene blue, 2-(N-phenyl-N-methylamino)-6-(N-p-tolyl-N-ethyl)aminofluoran, 2-anilino-3-methyl-6-(n-ethyl-p-tolino)fluoran, 3,6-dimethoxyfluoran, 3-(N,N-diethylamino)-5-methyl-7-(N,N-dibenzylamino)fluoran, 3-(N-cyclohexyl-N-methylamino)-6-methyl-7-anilinofluoran, 3-(N,N-diethylamino)-6-methyl-7-anilinofluoran, 3-(N,N-diethylamino)-6-methyl-7-xylidinofluoran, 3-(N,N-diethylamino)-6-methyl-7-chlorofluoran, 3-(N,N-diethylamino)-6-methoxy-7-aminofluoran, 3-(N,N-diethylamino)-7-(4-chloroanilino)fluoran, 3-(N,N-diethylamino)-7-chlorofluoran, 3-(N,N-diethylamino)-7-benzylaminofluoran, 3-(N,N-diethylamino)-6-methyl-7-anilinofluoran, 3-(N,N-diethylamino)-6-methyl-7-xylidinofluoran, 3-piperidino-6-methyl-7-anilinofluoran, 3-pyrolidino-6-methyl-7-anilinofluoran, 3,3-bis(1-ethyl-2-methylindol-3-yl)phthalide, 3,3-bis(1-n-butyl-2-methylin-

dol-3-yl)phthalide, 3,3-bis(p-dimethylaminophenyl)-6-dimethylaminophthalide, 3-(4-diethylamino-2-ethoxyphenyl)-3-(1-ethyl-2-methylindol-3-yl)-4-phthalide and 3-(4-diethylaminophenyl)-3-(1-ethyl-2-methylindol-3-yl)phthalide.

The amount of the dye undergoing discoloration with an acid or radical is preferably from 0.01 to 10% by weight based on the solid content of the image-recording layer.

<5> Polymerization Inhibitor

10 It is preferred to add a small amount of a thermal polymerization inhibitor to the image-recording layer according to the invention in order to inhibit undesirable thermal polymerization of the polymerizable compound (C) during the production or preservation of the image-recording layer.

15 The thermal polymerization inhibitor preferably includes, for example, hydroquinone, p-methoxyphenol, di-tert-butyl-p-cresol, pyrogallol, tert-butyl catechol, benzoquinone, 4,4'-thiobis(3-methyl-6-tert-butylphenol), 2,2'-methylenebis(4-methyl-6-tert-butylphenol) and N-nitroso-N-

20 phenylhydroxylamine aluminum salt. The amount of the thermal polymerization inhibitor added is preferably from about 0.01 to about 5% by weight based on the total solid content of the image-recording layer.

<6> Higher Fatty Acid Derivative

25 To the image-recording layer according to the invention, a higher fatty acid derivative, for example, behenic acid or behenic acid amide may be added to localize on the surface of the image-recording layer during a drying step after coating in order to avoid polymerization inhibition due to oxygen.

30 The amount of the higher fatty acid derivative added is preferably from about 0.1 to about 10% by weight based on the total solid content of the image-recording layer.

<7> Plasticizer

35 The image-recording layer according to the invention may contain a plasticizer in order to improve the on-press development property. The plasticizer preferably includes, for example, a phthalic acid ester, e.g., dimethyl phthalate, diethyl phthalate, dibutyl phthalate, diisobutyl phthalate, dioctyl phthalate, octyl capryl phthalate, dicyclohexyl phthalate,

40 ditridecyl phthalate, butyl benzyl phthalate, diisodecyl phthalate or diallyl phthalate; a glycol ester, e.g., dimethylglycol phthalate, ethylphthalylethyl glycolate, methylphthalylethyl glycolate, butylphthalylethyl glycolate or triethylene glycol dicaprylate ester; a phosphoric acid ester, e.g., tricresyl phosphate or triphenyl phosphate; an aliphatic dibasic acid ester,

45 e.g., diisobutyl adipate, dioctyl adipate, dimethyl sebacate, dibutyl sebacate, dioctyl azelate or dibutyl maleate; polyglycidyl methacrylate, triethyl citrate glycerin triacetyl ester and butyl laurate.

50 The amount of the plasticizer is preferably about 30% by weight or less based on the total solid content of the image-recording layer.

<8> Fine Inorganic Particle

55 The image-recording layer according to the invention may contain fine inorganic particle in order to increase the strength of cured film and to improve the on-press development property.

60 The fine inorganic particle preferably includes, for example, silica, alumina, magnesium oxide, titanium oxide, magnesium carbonate, calcium alginate and a Are thereof. The fine inorganic particle can be used, for example, for strengthening the film or enhancing interface adhesion property due to surface roughening.

65 The file inorganic particle preferably has an average particle size from 5 nm to 10  $\mu$ m, more preferably from 0.5 to 3  $\mu$ m. In the range described above, it is stably dispersed in the image-recording layer, sufficiently maintains the film

strength of the image-recording layer and can form the non-imaging area excellent in hydrophilicity and prevented from the occurrence of stain at the time of printing.

The fine inorganic particle described above is easily available as a commercial product, for example, colloidal silica dispersion.

The amount of the fine inorganic particle added is preferably 40% by weight or less, more preferably 30% by weight or less, based on the total solid content of the image-recording layer.

<9> Hydrophilic Low Molecular Weight Compound

The image-recording layer according to the invention may contain a hydrophilic low molecular weight compound in order to improve the on-press development property. The hydrophilic low molecular weight compound includes a water-soluble organic compound, for example, a glycol compound, e.g., ethylene glycol, diethylene glycol, triethylene glycol, propylene glycol, dipropylene glycol or tripropylene glycol, or an ether or ester derivative thereof, a polyhydroxy compound, e.g., glycerine or pentaerythritol, an organic amine compound, e.g., triethanol amine, diethanol amine or monoethanol amine, or a salt thereof, an organic sulfonic acid compound, e.g., an alkyl sulfonic acid, toluene sulfonic acid or benzene sulfonic acid, or a salt thereof, an organic sulfamic acid compound, e.g., an alkyl sulfamic acid, or a salt thereof, an organic sulfuric acid compound, e.g., an alkyl sulfuric acid or an alkyl ether sulfuric acid, or a salt thereof, an organic phosphonic acid compound, e.g., phenyl phosphonic acid, or a salt thereof, an organic carboxylic acid, e.g., tartaric acid, oxalic acid, citric acid, malic acid, lactic acid, gluconic acid or an amino acid, or a salt thereof.

Of the compounds, sodium salt or lithium salt of an organic sulfonic acid, organic sulfamic acid or organic sulfuric acid is preferably used. By incorporating the compound into the image-recording layer, it is possible to increase the on-press development property without accompanying the decrease in printing durability.

Specific examples of the salt of organic sulfonic acid include sodium n-butylsulfonate, sodium isobutylsulfonate, sodium sec-butylsulfonate, sodium tert-butylsulfonate, sodium n-pentylsulfonate, sodium 1-ethylpropylsulfonate, sodium n-hexylsulfonate, sodium 1,2-dimethylpropylsulfonate, sodium 2-ethylbutylsulfonate, sodium cyclohexylsulfonate, sodium n-heptylsulfonate, sodium n-octylsulfonate, sodium tert-octylsulfonate, sodium n-nonylsulfonate, sodium allylsulfonate, sodium 2-methylallylsulfonate, sodium benzenesulfonate, sodium p-toluenesulfonate, sodium p-hydroxybenzenesulfonate, sodium p-styrene-sulfonate, sodium isophthalic acid dimethyl-5-sulfonate, disodium 1,3-benzenedisulfonate, trisodium 1,3,5-benzenetrisulfonate, sodium p-chlorobenzenesulfonate, sodium 3,4-dichlorobenzenesulfonate, sodium 1-naphthylsulfonate, sodium 2-naphthylsulfonate, sodium 4-hydroxynaphthylsulfonate, disodium 1,5-naphthyldisulfonate, disodium 2,6-naphthyldisulfonate, trisodium 1,3,6-naphyltrisulfonate and lithium salts of these compounds wherein the sodium is exchanged with lithium.

Specific examples of the salt of organic sulfamic acid include sodium n-butylsulfamate, sodium isobutylsulfamate, sodium tert-butylsulfamate, sodium n-pentylsulfamate, sodium 1-ethylpropylsulfamate, sodium n-hexylsulfamate, sodium 1,2-dimethylpropylsulfamate, sodium 2-ethylbutylsulfamate, sodium cyclohexylsulfamate and lithium salts of these compounds wherein the sodium is exchanged with lithium.

The hydrophilic low molecular weight compound has the hydrophobic part of a small structure and almost no surface

active function so that it can be clearly distinguished from the surfactant described hereinbefore in which a long-chain alkylsulfonate or a long-chain alkylbenzenesulfonate is preferably used.

As the salt of organic sulfuric acid, a compound represented by formula (2) shown below is particularly preferably used.



15 In formula (2), R represents a substituted or unsubstituted allyl group, a substituted or unsubstituted alkenyl group, a substituted or unsubstituted alkynyl group, a substituted or unsubstituted aryl group or a substituted or unsubstituted heterocyclic group, m represents an integer of 1 to 4, and X represents sodium, potassium or lithium.

20 R in formula (2) preferably represents a substituted or unsubstituted, straight-chain, branched or cyclic alkyl group having from 1 to 12 carbon atoms, a substituted or unsubstituted alkenyl group having from 1 to 12 carbon atoms, a substituted or unsubstituted alkynyl group having from 1 to 12 carbon atoms or a substituted or unsubstituted aryl group having 20 or less carbon atoms. Examples of the substituent include a straight-chain, branched or cyclic alkyl group having from 1 to 12 carbon atoms, an alkenyl group having from 1 to 12 carbon atoms, an alkynyl group having from 1 to 12 carbon atoms, a halogen atom and an aryl group having 20 or less carbon atoms.

25 Preferable examples of the compound represented by formula (2) include sodium oxyethylene 2-ethylhexyl ether sulfate, sodium dioxyethylene 2-ethylhexyl ether sulfate, potassium dioxyethylene 2-ethylhexyl ether sulfate, lithium dioxyethylene 2-ethylhexyl ether sulfate, sodium trioxyethylene 2-ethylhexyl ether sulfate, sodium tetraoxyethylene 2-ethylhexyl ether sulfate, sodium dioxyethylene hexyl ether sulfate, sodium dioxyethylene octyl ether sulfate and sodium dioxyethylene lauryl ether sulfate. Most preferable examples thereof include sodium dioxyethylene 2-ethylhexyl ether sulfate, potassium dioxyethylene 2-ethylhexyl ether sulfate and lithium dioxyethylene 2-ethylhexyl ether sulfate.

30 As the hydrophilic low molecular weight compound, as well as the compounds described above, a compound having a specific isocyanuric acid skeleton represented by formula (3) shown below is also preferably used.



40 In formula (3), at least one of R<sup>1</sup> to R<sup>3</sup> represents a  $-(CH_2CH_2O)_n-R^4$  group, R<sup>4</sup> represents a hydrogen atom or an alkyl group having from 1 to 4 carbon atoms, n represents an integer of 1 to 20, the remainder of R<sup>1</sup> to R<sup>3</sup> each independently represents a group selected from a hydrogen atom, an alkyl group having from 1 to 4 carbon atoms and a  $-R^5-COOH$  group, and R<sup>5</sup> represents an alkylene group having from 1 to 6 carbon atoms.

49

Of the compounds having a specific isocyanuric acid skeleton for use in the invention, from the standpoint of on-press development efficiency, the compounds wherein two or more of R<sup>1</sup> to R<sup>3</sup> represent the —(CH<sub>2</sub>CH<sub>2</sub>O)<sub>n</sub>—R<sup>4</sup> groups are preferable and the compounds wherein all of R<sup>1</sup> to R<sup>3</sup> represent the —(CH<sub>2</sub>CH<sub>2</sub>O)<sub>n</sub>—R<sup>4</sup> groups are particularly preferable.

In the case where R<sup>4</sup> represents an alkyl group having from 1 to 4 carbon atoms, examples of the alkyl group include a methyl group, an ethyl group, a n-propyl group, an isopropyl group, an n-butyl group, an isobutyl group and a tert-butyl group.

Of the —(CH<sub>2</sub>CH<sub>2</sub>O)<sub>n</sub>—R<sup>4</sup> groups, from the standpoint of on-press development efficiency, n is preferably an integer of 1 to 10, more preferably an integer of 1 to 3, and R<sup>4</sup> is preferably a hydrogen atom or a methyl group, particularly preferably a hydrogen atom.

In the case where any one of R<sup>1</sup> to R<sup>3</sup> represents an alkyl group having from 1 to 4 carbon atoms, examples of the alkyl group include a methyl group, an ethyl group, a n-propyl group, an isopropyl group, an n-butyl group, an isobutyl group and a tert-butyl group. Among the alkyl groups, a methyl group and an ethyl group are preferable.

In the case where any one of R<sup>1</sup> to R<sup>3</sup> represents the —R<sup>5</sup>—COOH group, a —C<sub>2</sub>H<sub>4</sub>COOH group is preferably exemplified.

The remainder of R<sup>1</sup> to R<sup>3</sup> other than the —(CH<sub>2</sub>CH<sub>2</sub>O)<sub>n</sub>—R<sup>4</sup> group is preferably a hydrogen atom or a methyl group, particularly preferably a hydrogen atom.

Specific examples of the compounds having a specific isocyanuric acid skeleton for use in the invention include compounds represented by structural formulae (D-1) to (D-10) set forth below, but the invention should not be construed as being limited thereto.



50

-continued

(D-4)



60 Of the compounds described above, tris(2-hydroxyethyl) isocyanurate represented by structural formula (D-1) is particularly preferable, because the balance of acceleration of on-press development property and printing durability is especially excellent.

65 The amount of the hydrophilic low molecular weight compound added to the image-recording layer is preferably from 0.5 to 20% by weight more preferably from 1 to 10% by

51

weight, still more preferably from 2 to 8% by weight, based on the total solid content of the image-recording layer. In the range described above, good on-press development property and good printing durability are achieved.

The hydrophilic low molecular weight compounds may be used individually or as a mixture of two or more thereof.

<10> Oil-Sensitizing Agent

In the case where an inorganic stratiform compound is incorporated into a protective layer described hereinafter, it is preferred that a phosphonium compound is used together in order to improve an ink-receptive property. The phosphonium compound functions as a surface covering agent (oil-sensitizing agent) of the inorganic stratiform compound and prevents deterioration of the ink-receptive property during printing due to the inorganic stratiform compound.

As preferable examples of the phosphonium compound, compounds represented by formula (4) shown below and compounds represented by formula (5) shown below are exemplified. More preferable examples of the phosphonium compound include the compounds represented by formula (4).



In formula (4),  $\text{Ar}_1$  to  $\text{Ar}_6$  each independently represents an aryl group or a heterocyclic group,  $\text{L}$  represents a divalent connecting group,  $\text{X}^{n-}$  represents a  $n$ -valent counter anion,  $n$  represents an integer of 1 to 3, and  $n$  represents a number satisfying  $n \times m = 2$ .

The aryl group preferably includes, for example, a phenyl group, a naphthyl group, a tolyl group, a xylyl group, a fluorophenyl group, a chlorophenyl group, a bromophenyl group, a methoxyphenyl group, an ethoxyphenyl group, a dimethoxyphenyl group, a methoxycarbonylphenyl group and a dimethylaminophenyl group. The heterocyclic group preferably includes, for example, a pyridyl group, a quinolyl group, a pyridinyl group, a thieryl group and a furyl group.  $\text{L}$  preferably represents a divalent connecting group having from 6 to 15 carbon atoms, more preferably a divalent connecting group having from 6 to 12 carbon atoms.

$\text{X}^{n-}$  preferably represents a halogen anion, for example,  $\text{Cl}^-$ ,  $\text{Br}^-$  or  $\text{I}^-$ , a sulfonate anion, a carboxylate anion, a sulfate ester anion,  $\text{PF}_6^-$ ;  $\text{BF}_4^-$  and a perchlorate anion. Among them, a halogen anion, for example,  $\text{Cl}^-$ ,  $\text{Br}^-$  or  $\text{I}^-$ , a sulfonate anion and a carboxylate anion are particularly preferable.

52

Specific examples of the phosphonium compound represented by formula (4) are set forth below.



53  
-continued54  
-continued

55  
-continued56  
-continued

In formula (5),  $R_1$  to  $R_4$  each independently represents an alkyl group, an alkenyl group, an alkynyl group, a cycloalkyl group, an alkoxy group, an aryl group, an aryloxy group, an alkylthio group or a heterocyclic group, each of which may have a substituent; or a hydrogen atom, alternatively, at least two of  $R_1$  to  $R_4$  may be combined with each other to form a ring, and  $X^-$  represents a counter anion.

When any one of  $R_1$  to  $R_4$  represents an alkyl group, an alkoxy group or an alkylthio group, a number of carbon atoms included is ordinarily from 1 to 20. When any one of  $R_1$  to  $R_4$  represents an alkenyl group or an alkynyl group, a number of carbon atoms included is ordinarily from 2 to 15. When any one of  $R_1$  to  $R_4$  represents a cycloalkyl group, a number of carbon atoms included is ordinarily from 3 to 8. Examples of the aryl group include a phenyl group and a naphthyl group. Examples of the aryloxy group include a phenoxy group and a naphthoxy group. Examples of the arylthio group include a phenylthio group. Examples of the heterocyclic group include a furyl group and a thieryl group. Examples of the substituent for these groups include alkyl group, an alkenyl group, an alkynyl group, a cycloalkyl group, an alkoxy group, an alkoxy carbonyl group, an acyl group, an alkylthio group,

57

an aryl group, an aryloxy group, an arylthio group, a sulfino group, a sulfo group, a phosphino group, a phosphoryl group, an amino group, a nitro group, a cyano group, a hydroxy group and a halogen atom. The substituent may further have a substituent.

Examples of the anion represented by  $X^-$  include a halide ion, for example,  $Cl^-$ ,  $Br^-$  or  $I^-$ , an inorganic acid anion, for example,  $ClO_4^-$ ,  $PF_6^-$  or  $SO_4^{2-}$ , an organic carboxylic acid anion and an organic sulfonic acid anion. Examples of the organic group for the organic carboxylic acid anion and organic sulfonic acid anion include a methyl group, an ethyl group, a propyl group, a butyl group, a phenyl group, a methoxyphenyl group, a naphthyl group, a fluorophenyl group, a difluorophenyl group, a pentafluorophenyl group, a thiienyl group and a pyrrolyl group. Among them,  $Cl^-$ ,  $Br^-$ ;  $I^-$ ,  $ClO_4^-$  and  $PF_6^-$  are preferable.

Specific examples of the phosphonium compound represented by formula (5) are set forth below.



55

60

65

58

-continued



35

40

45

50

55

60

65

59

-continued



A nitrogen-containing low molecular weight compound described below is also exemplified as the oil-sensitizing agent which is preferably used in the invention as well as the phosphonium compound. Preferable examples of the nitrogen-containing low molecular weight compound include

60

compounds having a structure represented by formula (I) shown below.

5



(I)

10

In formula (1),  $\text{R}_1$  to  $\text{R}_4$  each independently represents an alkyl group, an alkenyl group, an alkynyl group, a cycloalkyl group, an alkoxy group, an aryl group, an aralkyl group or a heterocyclic group, each of which may have a substituent, or a hydrogen atom, alternatively, at least two of  $\text{R}_1$  to  $\text{R}_4$  may be combined with each other to form a ring, and  $\text{X}^-$  represents an anion including  $\text{PF}_6^-$ ,  $\text{BF}_4^-$  or an organic sulfonate anion having a substituent selected from an allyl group, an alkenyl group, an alkynyl group, a cycloalkyl group, an alkoxy group, an aryl group, an aralkyl group and a heterocyclic group.

Specifically, the nitrogen-containing low molecular weight compound for use in the invention includes an amine salt in which at least one of  $\text{R}_1$  to  $\text{R}_4$  in formula (I) is a hydrogen atom, a quaternary ammonium salt in which any of  $\text{R}_1$  to  $\text{R}_4$  in formula (II) is not a hydrogen atom. Also, it may have a structure of an imidazolinium salt represented by formula (II) shown below, of a benzimidazolinium salt represented by formula (III) shown below, of a pyridinium salt represented by formula (I) shown below, or of a quinolinium salt represented by formula (V) shown below.

35



(II)

40



(III)

45



(IV)

50



(V)

55

In the above formulae  $\text{R}_5$  and  $\text{R}_6$  each independently represents an alkyl group, an alkenyl group, an alkynyl group, a cycloalkyl group, an alkoxy group, an aryl group, an aralkyl group or a heterocyclic group, each of which may have a substituent or a hydrogen atom, and  $\text{X}^-$  represents an anion having the same meaning as  $\text{X}$  in formula (I).

Of the nitrogen-containing low molecular weight compounds, the quaternary ammonium salt and pyridinium salt are preferably used. Specific examples thereof are set forth below.



52

-continued



The amount of the phosphonium compound or nitrogen-containing low molecular weight compound added to the image-recording layer is preferably from 0.01 to 20% by weight, more preferably from 0.05 to 10% by weight, most preferably from 0.1 to 5% by weight, based on the solid

63

content of the image-recording layer. In the range described above, good ink-receptive property during printing is obtained.

As the oil-sensitizing agent for use in the invention, a polymer containing an ammonium group described below is also preferably exemplified. The polymer containing an ammonium group may be any polymer containing an ammonium group in its structure and is preferably a polymer containing as repeating units, a structure represented by formula (VI) shown below and a structure represented by formula (VII) shown below.



In formulae (VI) and (VII),  $\text{R}^{11}$  and  $\text{R}^{12}$  each independently represents a hydrogen atom or a methyl group,  $\text{R}^2$  represents a divalent connecting group, for example, an alkylene group which may have a substituent or all alkyleneoxy group which may have a substituent,  $\text{R}^{31}$ ,  $\text{R}^{32}$  and  $\text{R}^{33}$  each independently represents an alkyl group having from 1 to 20 carbon atoms or an aralkyl group,  $\text{X}^-$  represents an organic or inorganic anion, for example,  $\text{F}^-$ ,  $\text{Cl}^-$ ,  $\text{Br}^-$ ,  $\text{I}^-$ , a benzene-sulfonate anion which may have a substituent, a methylsulfate anion, an ethylsulfate anion, a propylsulfate anion, a butylsulfate anion which may be branched, an amylsulfate anion which may be branched,  $\text{PF}_6^-$ ,  $\text{BF}_4^-$  or  $\text{B}(\text{C}_6\text{F}_5)_4^-$ ;  $\text{R}^4$  represents an alkyl group having from 1 to 21 carbon atoms, an aralkyl group, an aryl group,  $-(\text{C}_2\text{H}_4\text{O})_n-\text{R}^5$  or  $-(\text{C}_3\text{H}_6\text{O})_n-\text{R}^5$ ,  $\text{R}^5$  represents a hydrogen atom, a methyl group or an ethyl group, and  $n$  represents 1 or 2.

The polymer containing an ammonium group includes at least one of the structural units represented by formula (V) and at least one of the structural units represented by formula (VII), and it may include two or more of the structural units represented by formula (VI) or (VII) or both. A ratio of the both structural units is not particularly restricted and is particularly preferably from 5:95 to 80:20. The polymer may include other copolymerization component within a range of ensuring the effects of the invention.

As to the polymer containing an ammonium group, a reduced specific viscosity value (unit: cSt/g/ml) obtained according to the measuring method described below is preferably from 5 to 120, more preferably from 10 to 110, particularly preferably from 15 to 100.

#### <Measuring Method of Reduced Specific Viscosity>

In a 20 ml measuring flask was weighed 3.33 g of a 30% by weight polymer solution (1 g as a solid content) and the measuring flask was fed up to the gauge line with *N*-methyl pyrrolidone. The resulting solution was put into an Ubbelohde viscometer (viscometer constant: 0.010 cSt/s) and a period for running down of the solution at 30° C. was mea-

64

sured. The viscosity was determined in a conventional manner according to the following calculating formula:

Kinetic viscosity=Viscometer constant×Period for liquid to pass through a capillary (sec)

5 The content of the polymer containing an ammonium group is preferably from 0.0005 to 30.0% by weight more preferably from 0.001 to 20.0% by weight, most preferably from 0.002 to 15.0% by weight, based on the total solid content of the image-recording layer. In the range described above, good ink-receptive property is obtained.

10 Specific examples of the polymer containing an ammonium group are set forth below.

Formula (VI)

15



Formula (VII)

25



(1)

(2)

(3)

(4)

(5)



**65**

-continued

**66**

-continued



**67**  
-continued



**68**  
-continued



(18) The oil-sensitizing agent may be added to a protective layer in addition to the image-recording layer.  
<Formation of Image-Recording Layer>

(19) The image-recording layer according to the invention is formed by dispersing or dissolving each of the necessary constituting components described above in a solvent to prepare a coating solution and coating the solution. The solvent used include for example, ethylene dichloride, cyclohexanone, methyl ethyl ketone, methanol, ethanol, propanol, ethylene glycol monomethyl ether, 1-methoxy-2-propanol, 2-methoxyethyl acetate, 1-methoxy-2-propyl acetate, dimethoxyethane, methyl lactate, ethyl lactate, N,N-dimethylacetamide, N,N-dimethylformamide, tetramethylurea, N-methylpyrrolidone, dimethylsulfoxide, sulfolane,  $\gamma$ -butyrolactone, toluene and water, but the invention should not be construed as being limited thereto. The solvents may be used individually or as a mixture. The solid content concentration of the coating solution is preferably from 1 to 50% by weight.

(20) The image-recording layer according to the invention may also be formed by preparing plural coating solutions by dispersing or dissolving the same or different components described above into the same or different solvents and conducting repeatedly the coating and drying plural times.

(21) The coating amount of the image-recording layer (solid content) formed on a support after drying may be varied according to the intended purpose but is preferably from 0.3 to 3.0 g/m<sup>2</sup>. In the range described above, good sensitivity and good film property of the image-recording layer can be

(22) achieved. Various methods can be used for the coating. Examples of the coating method include bar coater coating, spin coating, spray coating, curtain coating, dip coating, air knife coating, blade coating and roll coating.

(Protective Layer) (23) In the lithographic printing plate precursor according to the invention, it is preferable to provide a protective layer (over-coat layer) on the image-recording layer. The protective layer has a function for preventing, for example, occurrence of scratch in the image-recording layer or ablation caused by exposure with a high illuminance laser beam, in addition to the function for restraining an inhibition reaction against the image formation by means of oxygen blocking. The consti-

tuting components of the protective layer according to the invention will be described below.

Ordinarily, the exposure process of a lithographic printing plate precursor is performed in the air. The image-forming reaction occurred upon the exposure process in the image-recording layer may be inhibited by a low molecular weight compound, for example, oxygen or a basic substance present in the air. The protective layer prevents the low molecular weight compound, for example, oxygen or the basic substance from penetrating into the image-recording layer and as a result the inhibition reaction against the image formation at the exposure process in the air can be restrained. Accordingly, the property required of the protective layer is to reduce permeability of the low molecular compound, for example, oxygen. Further, the protective layer preferably has good transparency to light used for the exposure, is excellent in an adhesion property to the image-recording layer, and can be easily removed during the on-press development processing step after the exposure. With respect to the protective layer having such properties, there are described, for example, in U.S. Pat. No. 3,458,311 and JP-B-55-49729.

As a material for use in the protective layer, any water-soluble polymer and water-insoluble polymer can be appropriately selected to use. Specifically, a water-soluble polymer, for example, polyvinyl alcohol, a modified polyvinyl alcohol, polyvinyl pyrrolidone, polyvinyl imidazole, polyacrylic acid, polyacrylamide, a partially saponified product of polyvinyl acetate, an ethylene-vinyl alcohol copolymer, a water-soluble cellulose derivative, gelatin, a starch derivative or gum arabic, and a polymer, for example, polyvinylidene chloride, poly(meth)acrylonitrile, polysulfone, polyvinyl chloride, polyethylene, polycarbonate, polystyrene, polyamide or cellophane are exemplified. The polymers may be used in combination of two or more thereof, if desired.

As a relatively useful material for use in the protective layer, a water-soluble polymer compound excellent in crystallinity is exemplified. Specifically, polyvinyl alcohol, polyvinyl pyrrolidone, polyvinyl imidazole, a water-soluble acrylic resin, for example, polyacrylic acid, gelatin or gum arabic is preferably used. Above all, polyvinyl alcohol, polyvinyl pyrrolidone and polyvinyl imidazole are more preferably used from the standpoint of capability of coating with water as a solvent and easiness of removal with dampening water at the printing. Among them, polyvinyl alcohol (PVA) provides most preferable results on the fundamental properties, for example, oxygen blocking property or removability with development.

The polyvinyl alcohol for use in the protective layer may be partially substituted with ester, ether or acetal as long as it contains a substantial amount of unsubstituted vinyl alcohol units necessary for maintaining water solubility. Also, the polyvinyl alcohol may partially contain other copolymerization components. For instance, polyvinyl alcohols of various polymerization degrees having at random a various kind of hydrophilic modified cites, for example, an anion-modified cite modified with an anion, e.g., a carboxyl group or a sulfo group, a cation-modified cite modified with a cation, e.g., an amino group or an ammonium group, a silanol-modified cite or a thiol-modified cite, and polyvinyl alcohols of various polymerization degrees having at the terminal of the polymer chain a various kind of modified cites, for example, the above-described anion-modified cite, cation modified cite, silanol-modified cite or thiol-modified cite, an alkoxy-modified cite, a sulfide-modified cite, an ester modified cite of vinyl alcohol with a various kind of organic acids, an ester modified cite of the above-described anion-modified cite with an alcohol or an epoxy-modified cite are also preferably used.

Preferable examples of the polyvinyl alcohol include those having a hydrolysis degree of 71 to 100% by mole and a polymerization degree of 300 to 2,400. Specific examples of the polyvinyl alcohol include PVA-105, PVA-110, PVA-117, PVA-117H PVA-120, PVA-124, PVA-124H, PVA-CS, PVA-CST, PVA-HC, PVA-203, PVA-204, PVA-205, PVA-210, PVA-217, PVA-220, PVA-224, PVA-217EE, PVA-217F, PVA-220E, PVA-224E, PVA-405, PVA-420, PVA-613 and L-8, produced by Kuraray Co., Ltd.

Specific examples of the modified polyvinyl alcohol include that having an anion-modified cite, for example, KL-318, KL-118, KM-618, KM-118 or SK-5102, that having a cation-modified cite, for example, C-318, C-118 or CM-318, that having a terminal thiol-modified cite, for example, M-205 or M-115, that having a terminal sulfide-modified cite, for example, MP-103, MP-203, NT-102 or MP-202, that having an ester-modified cite with a higher fatty acid at the terminal, for example, EL-12E or DL-1203 and that having a reactive silane-modified cite, for example, R-1130, R-2105 or R-2130, produced by Kuraray Co., Ltd.

It is also preferable that the protective layer contains an inorganic stratiform compound. The stratiform compound is a particle having a thin tabular shape and includes, for instance, mica, for example, natural mica represented by the following formula: A (B, C)<sub>2-5</sub> D<sub>4</sub> O<sub>10</sub> (OH, F, O)<sub>2</sub>, (wherein A represents any one of Li, K, Na, Ca, Mg and an organic cation, B and C each represents any one of Fe(II), Fe(III), Mn, Al, Mg and V, and D represents Si or Al) or synthetic mica, talc represented by the following formula: 3MgO.4SiO<sub>2</sub>H<sub>2</sub>O, teniolite, montmorillonite, saponite, hecolite and zirconium phosphate.

Examples of the natural mica include muscovite, paragonite, phlogopite, biotite and lepidolite. Examples of the synthetic mica include non-swellable mica, for example, fluor-phlogopite KMg<sub>3</sub>(AlSi<sub>3</sub>O<sub>10</sub>)F<sub>2</sub> or potassium tetrasilic mica KMg<sub>2.5</sub>(Si<sub>4</sub>O<sub>10</sub>)F<sub>2</sub>, and swellable mica, for example, Na tetrasilic mica NaMg<sub>2.5</sub>(Si<sub>4</sub>O<sub>10</sub>)F<sub>2</sub>, Na or Li teniolite (Na, Li)Mg<sub>2</sub>Li(Si<sub>4</sub>O<sub>10</sub>)F<sub>2</sub>, or montmorillonite based Na or Li hecolite (Na, Li)<sub>1/8</sub>Mg<sub>2/5</sub>Li<sub>1/8</sub>(Si<sub>4</sub>O<sub>10</sub>)F<sub>2</sub>. Synthetic smectite is also useful.

Of the stratiform compounds, fluorine-based swellable mica, which is a synthetic stratiform compound, is particularly useful in the invention. Specifically, the swellable synthetic mica and an swellable clay mineral, for example, montmorillonite, saponite, hecolite or bentonite have a stratiform structure comprising a unit crystal lattice layer having thickness of approximately 10 to 15 angstroms, and metallic atom substitution in the lattices thereof is remarkably large in comparison with other clay minerals. As a result the lattice layer results in lack of positive charge and to compensate it, a cation, for example, Li<sup>+</sup>, Na<sup>+</sup>, Ca<sup>2+</sup>, Mg<sup>2+</sup> or an organic cation, e.g., an amine salt a quaternary ammonium salt a phosphonium salt or a sulfonium salt is adsorbed between the lattice layers. The stratiform compound swells upon contact with water. When share is applied under such condition the stratiform crystal lattices are easily cleaved to form a stable sol in water. The bentnite and swellable synthetic mica have strongly such tendency.

With respect to the shape of the stratiform compound, the thinner the thickness or the larger the plain size as long as smoothness of coated surface and transmission of actinic radiation are not damaged, the better from the standpoint of control of diffusion. Therefore, an aspect ratio of the stratiform compound is ordinarily 20 or more, preferably 100 or more, particularly preferably 200 or more. The aspect ratio is a ratio of thickness to major axis of particle and can be

determined, for example, from a projection drawing of particle by a microphotography. The larger the aspect ratio, the greater the effect obtained.

As for the particle diameter of the stratiform compound, an average diameter is ordinarily from 0.3 to 20  $\mu\text{m}$ , preferably from 0.5 to 10  $\mu\text{m}$ , particularly preferably from 1 to 5  $\mu\text{m}$ . When the particle diameter is less than 0.3  $\mu\text{m}$ , the inhibition of permeation of oxygen or moisture is insufficient and the effect of the stratiform compound can not be satisfactorily achieved. On the other hand, when it is larger than 20  $\mu\text{m}$ , the dispersion stability of the particle in the coating solution is insufficient to cause a problem in that stable coating can not be performed. An average thickness of the particle is ordinarily 0.1  $\mu\text{m}$  or less, preferably 0.05  $\mu\text{m}$  or less, particularly preferably 0.01  $\mu\text{m}$  or less. For example, with respect to the swellable synthetic mica that is the representative compound of the inorganic stratiform compounds, the thickness is approximately from 1 to 50 nm and the plain size is approximately from 1 to 20  $\mu\text{m}$ .

When such an inorganic stratiform compound particle having a large aspect ratio is incorporated into the protective layer, strength of the coated layer increases and penetration of oxygen or moisture can be effectively inhibited so that the protective layer can be prevented from deterioration due to deformation, and even when the lithographic printing plate precursor is preserved for a long period of time under a high humidity condition, it is prevented from decrease in the image-forming property thereof due to the change of humidity and exhibits excellent preservation stability.

An example of common dispersing method for using the stratiform compound in the protective layer is described below. Specifically, from 5 to 10 parts by weight of a swellable stratiform compound which is exemplified as a preferable stratiform compound is added to 100 parts by weight of water to adapt the compound to water and to be swollen, followed by dispersing using a dispersing machine. The dispersing machine used include, for example, a variety of mills conducting dispersion by directly applying mechanical power, a high-speed agitation type dispersing machine providing a large shear force and a dispersion machine providing ultrasonic energy of high intensity. Specific examples thereof include a ball mill, a sand grinder mill, a visco mill, a colloid mill, a homogenizer, a dissolver, a polytron, a homomixer, a homoblender, a kiddy mill, a jet agitor; a capillary type emulsifying device, a liquid siren, an electromagnetic strain type ultrasonic generator and an emulsifying device having Polman whistle. A dispersion containing from 5 to 10% by weight of the inorganic stratiform compound thus prepared is highly viscous or gelled and exhibits extremely good preservation stability. In the formation of a coating solution for protective layer using the dispersion, it is preferred that the dispersion is diluted with water, sufficiently stirred and then mixed with a binder solution.

The content of the inorganic stratiform compound in the protective layer is ordinarily from 5/1 to 1/100 in terms of a weight ratio of the inorganic stratiform compound to an amount of a binder used in the protective layer. When a plural kind of the inorganic stratiform compounds is used together, it is preferred that the total amount of the inorganic stratiform compounds is in the range of weight ratio described above.

The inorganic stratiform compound can be added to the image-recording layer in addition to the protective layer. The addition of inorganic stratiform compound to the image-recording layer is useful for improvements in the printing durability, polymerization efficiency (sensitivity) and time-lapse stability.

The amount of the inorganic stratiform compound added to the image-recording layer is preferably from 0.1 to 50% by weight more preferably from 0.3 to 30% by weight, most preferably from 1 to 10% by weight, based on the solid content of the image-recording layer.

As other additive for the protective layer, glycerol, dipropylene glycol or the like can be added in an amount corresponding to several % by weight of the water-soluble or water-insoluble polymer to impart flexibility. Further, an anionic surfactant, for example, sodium alkyl sulfate or sodium alkyl sulfonate; an amphoteric surfactant, for example, alkylaminocarboxylate or alkylaminodicarboxylate; or a non-ionic surfactant, for example, polyoxyethylene alkyl phenyl ether can be added. The amount of the surfactant added is from 0.1 to 100% by weight of the water-soluble or water-insoluble polymer.

Further, for the purpose of improving the adhesion property to the image-recording layer, for example, it is described in JP-A-49-70702 and BP-A-1,303,578 that sufficient adhesion can be obtained by mixing from 20 to 60% by weight of an acrylic emulsion, a water-insoluble vinyl pyrrolidone-vinyl acetate copolymer or the like in a hydrophilic polymer mainly comprising polyvinyl alcohol and coating the mixture on the image-recording layer. In the invention, any of such known techniques can be used.

Moreover, other functions can also be provided to the protective layer. For instance, by adding a coloring agent (for example, a water-soluble dye), which is excellent in permeability for infrared ray used for the exposure and capable of efficiently absorbing light at other wavelengths, a safe light adaptability can be improved without causing decrease in the sensitivity.

The formation of protective layer is performed by coating a coating solution for protective layer prepared by dispersing or dissolving the components of protective layer in a solvent on the image-recording layer, followed by drying. The coating solvent may be appropriately selected in view of the binder used, and when a water-soluble polymer is used, distilled water or purified water is preferably used as the solvent.

To the coating solution for protective layer can be added known additives, for example, an anionic surfactant, a non-ionic surfactant, a cationic surfactant or a fluorine-based surfactant for improving coating property or a water-soluble plasticizer for improving physical property of the coated layer. Examples of the water-soluble plasticizer include propionamide, cyclohexanediol, glycerin or sorbitol. Also, a water-soluble (meth)acrylic polymer can be added. Further, to the coating solution for protective layer may be added known additives for increasing an adhesion property to the image-recording layer or for improving time-lapse stability of the coating solution.

A coating method of the protective layer is not particularly limited, and known methods, for example, methods described in U.S. Pat. No. 3,458,311 and JP-B-55-49729 can be utilized. Specific examples of the coating method for the protective layer include a blade coating method, an air knife coating method, a gravure coating method, a roll coating method, a spray coating method, a dip coating method and a bar coating method.

The coating amount of the protective layer is preferably in a range from 0.01 to 10  $\text{g}/\text{m}^2$ , more preferably in a range from 0.02 to 3  $\text{g}/\text{m}^2$ , most preferably in a range from 0.02 to 1  $\text{g}/\text{m}^2$ , in terms of the coating amount after drying.

(Support) The support for use in the lithographic printing plate precursor according to the invention is not particularly restricted as long as it is a dimensionally stable plate-like material. The

support includes, for example, paper, paper laminated with plastic (for example, polyethylene, polypropylene or polystyrene), a metal plate (for example, aluminum, zinc or copper plate), a plastic film (for example, cellulose diacetate, cellulose triacetate, cellulose propionate, cellulose butyrate, cellulose acetate butyrate, cellulose nitrate, polyethylene terephthalate, polyethylene, polystyrene, polypropylene, polycarbonate or polyvinyl acetal film) and paper or a plastic film laminated or deposited with the metal described above. Preferable examples of the support include a polyester film and an aluminum plate. Among them, the aluminum plate is preferred since it has good dimensional stability and is relatively inexpensive.

The aluminum plate includes a pure aluminum plate, an alloy plate comprising aluminum as a main component and containing a trace amount of hetero elements and a thin film of aluminum or aluminum alloy laminated with plastic. The hetero element contained in the aluminum alloy includes, for example, silicon, iron, manganese copper, magnesium, chromium, zinc, bismuth, nickel and titanium. The content of the hetero element in the aluminum alloy is preferably 10% by weight or less. Although a pure aluminum plate is preferred in the invention, since completely pure aluminum is difficult to be produced in view of the refining technique, the aluminum plate may slightly contain the hetero element. The composition is not specified for the aluminum plate and those materials conventionally known and used can be appropriately utilized.

The thickness of the support is preferably from 0.1 to 0.6 mm, more preferably from 0.15 to 0.4 mm.

In advance of the use of aluminum plate, a surface treatment for example, roughening treatment or anodizing treatment is preferably performed. The surface treatment facilitates improvement in the hydrophilic property and ensure for adhesion property between the image-recording layer and the support. Prior to the roughening treatment of the aluminum plate, a degreasing treatment for example, with a surfactant, an organic solvent or an aqueous alkaline solution is conducted for removing rolling oil on the surface thereof, if desired.

The roughening treatment of the surface of the aluminum plate is conducted by various methods and includes, for example, mechanical roughening treatment, electrochemical roughening treatment (roughening treatment of electrochemically dissolving the surface) and chemical roughening treatment (roughening treatment of chemically dissolving the surface selectively).

As the method of the mechanical roughening treatment, a known method, for example, ball graining, brush graining, blast graining or buff graining can be used. Also, a transfer method can be employed wherein using a roll having concavo-convex shape the concavo-convex shape is transferred to the surface of aluminum plate during a rolling step of the aluminum plate.

The electrochemical roughening treatment method includes, for example, a method of conducting by passing alternating current or direct current in an electrolytic solution containing an acid, for example, hydrochloric acid or nitric acid. Also, a method of using a mixed acid described in JP-A-54-63902 can be exemplified.

The aluminum plate subjected to the roughening treatment is subjected, if desired, to an alkali etching treatment using an aqueous solution, for example, of potassium hydroxide or sodium hydroxide and further subjected to a neutralizing treatment, and then subjected to an anodizing treatment for improving the abrasion resistance, if desired.

As the electrolyte used for the anodizing treatment of the aluminum plate, various electrolytes capable of forming porous oxide film can be used. Ordinarily, sulfuric acid, hydrochloric acid, oxalic acid, chromic acid or a mixed acid thereof is used. The concentration of the electrolyte can be appropriately determined depending on the kind of the electrolyte used.

Since the conditions for the anodizing treatment are varied depending on the electrolyte used, they cannot be defined commonly. However, it is ordinarily preferred that electrolyte concentration in the solution is from 1 to 80% by weight, liquid temperature is from 5 to 70°C., current density is from 5 to 60 A/dm<sup>2</sup>, voltage is from 1 to 100 V, and electrolysis time is from 10 seconds to 5 minutes. The amount of the anodized film formed is preferably from 1.0 to 5.0 g/m<sup>2</sup>, more preferably from 1.5 to 4.0 g/m<sup>2</sup>. In the range described above, good printing durability and good scratch resistance in the non-image area of lithographic printing plate can be achieved.

The aluminum plate subjected to the surface treatment and having the anodized film as described above is used as it is as the support in the invention. However, in order to more improve the adhesion property to a layer provided thereon, hydrophilicity, stain resistance, heat insulating property or the like, other treatment, for example, an enlarging treatment of micropores or a sealing treatment of micropores of the anodized film described in JP-A-2001-253181 and JP-A-2001-322365, or a surface hydrophilizing treatment by immersing in an aqueous solution containing a hydrophilic compound may be appropriately conducted. Needless to say, the enlarging treatment and sealing treatment are not limited to those described in the above-described patents and any conventionally known method may be employed. For instance, as the sealing treatment; as well as a sealing treatment with steam, a sealing treatment with fluorozirconic acid alone, a sealing treatment with sodium fluoride or a sealing treatment with steam having added thereto lithium chloride may be employed.

The sealing treatment for use in the invention is not particularly limited and conventionally known methods can be employed. Among them, a sealing treatment with an aqueous solution containing inorganic fluorine compound, a sealing treatment with water vapor and a sealing treatment with hot water are preferred. The sealing treatments will be described in more detail below, respectively.

<1> Sealing Treatment With Aqueous Solution Containing Inorganic Fluorine Compound

As the inorganic fluorine compound used in the sealing treatment with an aqueous solution containing an inorganic fluorine compound, a metal fluoride is preferably exemplified.

Specific examples thereof include sodium fluoride, potassium fluoride, calcium fluoride, magnesium fluoride, sodium fluorozirconate, potassium fluorozirconate, sodium fluorotitanate, potassium fluorotitanate, ammonium fluorozirconate, ammonium fluorotitanate, potassium fluorotitanate, fluorozirconic acid, fluorotitanic acid, hexafluorosilicic acid, nickel fluoride, iron fluoride, fluorophosphoric acid and ammonium fluorophosphate. Among them, sodium fluorozirconate, sodium fluorotitanate, fluorozirconic acid and fluorotitanic acid are preferred.

The concentration of the inorganic fluorine compound in the aqueous solution is preferably 0.01% by weight or more, more preferably 0.05% by weight or more, in view of performing satisfactory sealing of micropores of the anodized film and it is preferably 1% by weight or less, more preferably 0.5% by weight or less, in view of the stain resistance.

The aqueous solution containing an inorganic fluorine compound preferably further contains a phosphate compound. When the phosphate compound is contained, the hydrophilicity on the anodized film surface is increased and thus, the on-press development property and stain resistance can be improved.

Preferable examples of the phosphate compound include phosphates of metal, for example, an alkali metal or an alkaline earth metal.

Specific examples of the phosphate compound include zinc phosphate, aluminum phosphate, ammonium phosphate, diammonium hydrogen phosphate, ammonium dihydrogen phosphate, monoammonium phosphate, monopotassium phosphate, monosodium phosphate, potassium dihydrogen phosphate, dipotassium hydrogen phosphate, calcium phosphate, sodium ammonium hydrogen phosphate, magnesium hydrogen phosphate, magnesium phosphate, ferrous phosphate, ferric phosphate, sodium dihydrogen phosphate, sodium phosphate, disodium hydrogen phosphate, lead phosphate, diammonium phosphate, calcium dihydrogen phosphate, lithium phosphate, phosphotungstic acid, ammonium phosphotungstate, sodium phosphotungstate, ammonium phosphomolybdate, sodium phosphomolybdate, sodium phosphate, sodium tripolyphosphate and sodium pyrophosphate. Among them, sodium dihydrogen phosphate, disodium hydrogen phosphate, potassium dihydrogen phosphate and dipotassium hydrogen phosphate are preferred.

The combination of the inorganic fluorine compound and the phosphate compound is not particularly limited, but it is preferred that the aqueous solution contains at least sodium fluorozirconate as the inorganic fluorine compound and at least sodium dihydrogen phosphate as the phosphate compound.

The concentration of the phosphate compound in the aqueous solution is preferably 0.01% by weight or more, more preferably 0.1% by weight or more, in view of improvement in the on-press development property and stain resistance, and it is preferably 20% by weight or less, more preferably 5% by weight or less, in view of solubility.

The ratio of respective compounds in the aqueous solution is not particularly limited, and the weight ratio between the inorganic fluorine compound and the phosphate compound is preferably from 1/200 to 10/1, more preferably from 1/30 to 2/1.

The temperature of the aqueous solution is preferably 20°C. or more, more preferably 40°C. or more, and it is preferably 100°C. or less, more preferably 80°C. or less.

The pH of the aqueous solution is preferably 1 or more, more preferably 2 or more, and it is preferably 11 or less, more preferably 5 or less.

A method of the sealing treatment with the aqueous solution containing an inorganic fluorine compound is not particularly limited and examples thereof include a dipping method and a spray method. One of the treatments may be used alone once or multiple times, or two or more thereof may be used in combination.

In particular, the dipping method is preferred. In the case of performing the treatment using the dipping method, the treating time is preferably one second or more, more preferably 3 seconds or more, and it is preferably 100 seconds or less, more preferably 20 seconds or less.

#### <2> Sealing Treatment With Water Vapor

Examples of the sealing treatment with water vapor include a method of continuously or discontinuously bringing water vapor under applied pressure or normal pressure into contact with the anodized film.

The temperature of the water vapor is preferably 80°C. or more, more preferably 95°C. or more, and it is preferably 105°C. or less.

The pressure of the water vapor is preferably in a range from (atmospheric pressure -50 mmAg) to (atmospheric pressure +300 mmAg) (from  $1.008 \times 10^5$  to  $1.043 \times 10^5$  Pa).

The time period for which water vapor is contacted is preferably one second or more, more preferably 3 seconds or more, and it is preferably 100 seconds or less, more preferably 20 seconds or less.

#### <3> Sealing Treatment With Hot Water

Examples of the sealing treatment with hot water include a method of dipping the aluminum plate having formed thereon the anodized film in hot water.

The hot water may contain an inorganic salt (for example, a phosphate) or an organic salt.

The temperature of the hot water is preferably 80°C. or more, more preferably 95°C. or more, and it is preferably 1000°C. or less.

The time period for which the aluminum plate is dipped in the hot water is preferably one second or more, more preferably 3 seconds or more, and it is preferably 100 seconds or less, more preferably 20 seconds or less.

The hydrophilizing treatment includes an alkali metal silicate method described in U.S. Pat. Nos. 2,714,066, 3,181,461, 3,280,734 and 3,902,734. In the method, the support is subjected to immersion treatment or electrolytic treatment in an aqueous solution containing, for example, sodium silicate.

In addition, the hydrophilizing treatment includes, for example, a method of treating with potassium fluorozirconate described in JP-B-36-22063 and a method of treating with polyvinyl phosphonic acid described in U.S. Pat. Nos. 3,276,868, 4,153,461, and 4,689,272.

In the case of using a support having a surface of insufficient hydrophilicity, for example, a polyester film, in the invention, it is desirable to coat a hydrophilic layer thereon to make the surface sufficiently hydrophilic. Examples of the hydrophilic layer preferably includes a hydrophilic layer

formed by coating a coating solution containing a colloid of

oxide or hydroxide of at least one element selected from beryllium, magnesium, aluminum, silicon, titanium, boron, germanium, tin, zirconium, iron, vanadium, antimony and a transition metal described in JP-A-2001-199175, a hydro-

philic layer containing an organic hydrophilic matrix obtained by crosslinking or pseudo-crosslinking of an organic hydrophilic polymer described in JP-A-2002-79772, a hydrophilic layer containing an inorganic hydrophilic matrix obtained by sol-gel conversion comprising hydrolysis and condensation reaction of polyalkoxysilane and titanate, zirconate or aluminate, and a hydrophilic layer comprising an inorganic thin layer having a surface containing metal oxide.

Among them, the hydrophilic layer formed by coating a coating solution containing a colloid of oxide or hydroxide of silicon is preferred.

Further, in the case of using, for example, a polyester film as the support in the invention, it is preferred to provide an antistatic layer on the hydrophilic layer side, opposite side to the hydrophilic layer or both sides. When the antistatic layer is provided between the support and the hydrophilic layer, it also contributes to improve the adhesion property of the hydrophilic layer to the support. As the antistatic layer, a polymer layer having fine particles of metal oxide or a matting agent dispersed therein described in JP-A-2002-79772 can be used.

The support preferably has a center line average roughness of 0.10 to 1.2  $\mu\text{m}$ . In the range described above, good adhe-

sion property to the image-recording layer, good printing durability and good stain resistance can be achieved.  
(Backcoat Layer)

After applying the surface treatment to the support or forming an undercoat layer described hereinafter on the support, a backcoat layer can be provided on the back surface of the support, if desired.

The backcoat layer preferably includes, for example, a coating layer comprising an organic polymer compound described in JP-A-5-45885 and a coating layer comprising a metal oxide obtained by hydrolysis and polycondensation of an organic metal compound or an inorganic metal compound described in JP-A-6-34174. Among them, use of an alkoxy compound of silicon, for example,  $\text{Si}(\text{OCH}_3)_4$ ,  $\text{Si}(\text{OC}_2\text{H}_5)_4$ ,  $\text{Si}(\text{OC}_3\text{H}_7)_4$  or  $\text{Si}(\text{OC}_4\text{H}_9)_4$  is preferred since the starting material is inexpensive and easily available.

(Undercoat Layer)

In the lithographic printing plate precursor, particularly, the lithographic printing plate precursor of on-press development type, according to the invention, an undercoat layer is provided between the support and the image-recording layer, if desired. The undercoat layer makes removal of the image-recording layer from the support in the unexposed area easy so that the on-press development property can be improved. Further, it is advantageous that in the case of infrared laser exposure, since the undercoat layer acts as a heat insulating layer, heat generated upon the exposure does not diffuse into the support and is efficiently utilized so that increase in sensitivity can be achieved.

As a compound for the undercoat layer (undercoat compound), specifically, for example, a silane coupling agent having an addition-polymerizable ethylenic double bond reactive group described in JP-A-10-282679 and a phosphorus compound having an ethylenic double bond reactive group described in JP-A-2-304441 are preferably exemplified.

As the most preferable undercoat compound, a polymer resin obtained by copolymerization of a monomer having an adsorbing group, a monomer having a hydrophilic group and a monomer having a crosslinkable group is exemplified.

The essential component of the polymer resin for undercoat layer is an adsorbing group to the hydrophilic surface of the support. Whether adsorptivity to the hydrophilic surface of the support is present or not can be judged, for example, by the following method.

A test compound is dissolved in an easily soluble solvent to prepare a coating solution, and the coating solution is coated and dried on a support so as to have the coating amount after drying of  $30 \text{ mg/m}^2$ . After thoroughly washing the support coated with the test compound using the easily soluble solvent the residual amount of the test compound that has not been removed by the washing is measured to calculate the adsorption amount of the test compound to the support. For measuring the residual amount, the residual amount of the test compound may be directly determined, or may be calculated by determining the amount of the test compound dissolved in the washing solution. The determination for the test compound can be performed, for example, by X-ray fluorescence spectrometry measurement reflection absorption spectrometry measurement or liquid chromatography measurement. The compound having the adsorptivity to support is a compound that remains by  $1 \text{ mg/m}^2$  or more even after conducting the washing treatment described above.

The adsorbing group to the hydrophilic surface of the support is a functional group capable of forming a chemical bond (for example, an ionic bond, a hydrogen bond, a coordinate bond or a bond with intermolecular force) with a substance

(for example, metal or metal oxide) or a functional group (for example, a hydroxy group) present on the hydrophilic surface of the support. The adsorbing group is preferably an acid group or a cationic group.

5 The acid group preferably has an acid dissociation constant (pKa) of 7 or less. Examples of the acid group include a phenolic hydroxy group, a carboxyl group,  $-\text{SO}_3\text{H}$ ,  $-\text{OSO}_3\text{H}$ ,  $-\text{PO}_3\text{H}_2$ ,  $-\text{OPO}_3\text{H}_2$ ,  $-\text{CONHSO}_2$ ,  $-\text{SO}_2\text{NHSO}_2$  and  $-\text{COCH}_2\text{COCH}_3$ . Among them,  $-\text{OPO}_3\text{H}_2$  and  $-\text{PO}_3\text{H}_2$  are particularly preferred. The acid group may be the form of a metal salt.

10 The cationic group is preferably an onium group. Examples of the onium group include an ammonium group, a phosphonium group, an arsonium group, a stibonium group, an oxonium group, a sulfonium group, a selenonium group, a stannonium group and iodonium group. Among them, the ammonium group, phosphonium group and sulfonium group are preferred, the ammonium group and phosphonium group are more preferred, and the ammonium group is most preferred.

15 20 Particularly preferable examples of the monomer having the adsorbing group include a compound represented by the following formula (U1) or (U2):



30 35 In formulae (U1) and (U2),  $\text{R}^1$ ,  $\text{R}^2$  and  $\text{R}^3$  each independently represents a hydrogen atom, halogen atom or an alkyl group having from 1 to 6 carbon atoms.  $\text{R}^1$ ,  $\text{R}^2$  and  $\text{R}^3$  each 40 independently represents preferably a hydrogen atom or an alkyl group having from 1 to 6 carbon atoms, more preferably a hydrogen atom or an alkyl group having from 1 to 3 carbon atoms, most preferably a hydrogen atom or a methyl group. It is particularly preferred that  $\text{R}^2$  and  $\text{R}^3$  each represents a hydrogen atom.  $\text{Z}$  represents a functional group adsorbing to the hydrophilic surface of the support.

45 In formula (U1),  $\text{X}$  represents an oxygen atom ( $-\text{O}-$ ) or imino group ( $-\text{NH}-$ ). Preferably,  $\text{X}$  represents an oxygen atom. In formula (U1),  $\text{L}$  represents a divalent connecting group. It is preferred that  $\text{L}$  represents a divalent aliphatic group (for example, an alkylene group, a substituted alkylene group, an alkenylene group, a substituted alkenylene group, an alkinylene group or a substituted alkinylene group), a 50 divalent aromatic group (for example, an arylene group or a substituted arylene group), a divalent heterocyclic group or a combination of each of these groups described above with an oxygen atom ( $-\text{O}-$ ), a sulfur atom ( $-\text{S}-$ ), an imino group ( $-\text{NH}-$ ), a substituted imino group ( $-\text{NR}-$ , where  $\text{R}$  represents an aliphatic group, an aromatic group or a heterocyclic group) or a carbonyl group ( $-\text{CO}-$ ).

55 The divalent aliphatic group may form a cyclic structure or a branched structure. The number of carbon atoms of the divalent aliphatic group is preferably from 1 to 20, more preferably from 1 to 15, most preferably from 1 to 10. It is preferred that the divalent aliphatic group is a saturated aliphatic group rather than an unsaturated aliphatic group. The

79

divalent aliphatic group may have a substituent. Examples of the substituent include a halogen atom, a hydroxy group, an aromatic group and a heterocyclic group.

The number of carbon atoms of the divalent aromatic group is preferably from 6 to 20, more preferably from 6 to 15, most preferably from 6 to 10. The divalent aromatic group may have a substituent. Examples of the substituent include a halogen atom, a hydroxy group, an aliphatic group, an aromatic group and a heterocyclic group

It is preferred that the divalent heterocyclic group has a 5-membered or 6-membered ring as the hetero ring. Other heterocyclic ring, an aliphatic ring or an aromatic ring may be condensed to the heterocyclic ring. The divalent heterocyclic group may have a substituent. Examples of the substituent include a halogen atom, a hydroxy group, an oxo group (=O), a thioxo group (=S), an imino group (=NH), a substituted imino group (=N—R, where R represents an aliphatic group, an aromatic group or a heterocyclic group), an aliphatic group, an aromatic group and a heterocyclic group.

It is preferred that L represents a divalent connecting group containing a plurality of polyoxyalkylene structures. It is more preferred that the polyoxyalkylene structure is a polyoxyethylene structure. Specifically, it is preferred that L contains  $—(OCH_2CH_2)_n—$  (n is an integer of 2 or more).

In formula (U2), Y represents a carbon atom or a nitrogen atom. In the case where Y is a nitrogen atom and L is connected to Y to form a quaternary pyridinium group, Z is not mandatory and may represent a hydrogen atom because the quaternary pyridinium group itself exhibits the adsorptivity. L represents a divalent connecting group same as in formula (U1) or a single bond.

With respect to the adsorbing functional group, the above description on the adsorbing group can be referred to.

Representative examples of the compound represented by formula (U1) or (U2) are set forth below.



60 The hydrophilic group in the polymer resin for undercoat layer which can be used in the invention preferably includes, for example, a hydroxy group, a carboxyl group, a carboxylate group, a hydroxyethyl group, a polyoxyethyl group, a hydroxypropyl group, a polyoxypropyl group, an amino group, an aminoethyl group, an aminopropyl group, an ammonium group, an amido group, a carboxymethyl group, a sulfonic acid group and a phosphoric acid group. Among

80

-continued



them, a sulfonic acid group exhibiting a highly hydrophilic property is preferable. Specific examples of the monomer having a sulfo group include a sodium salt or amine salt of methallyloxybenzenesulfonic acid, allyloxybenzenesulfonic acid, allylsulfonic acid, vinylsulfonic acid, p-styrenesulfonic acid, methallylsulfonic acid, acrylamido-tert-butylsulfonic acid, 2-acrylamido-2-methylpropanesulfonic acid or (3-acryloyloxypropyl)butylsulfonic acid. Among them from the standpoint of the hydrophilic property and handling property in the synthesis thereof, sodium salt of 2-acrylamido-acid is preferable.

It is preferred that the water-soluble polymer resin for undercoat layer according to the invention has a crosslinkable group. The crosslinkable group acts to improve the adhesion property to the image area. In order to impart the crosslinking property to the polymer resin for undercoat layer, introduction of a crosslinkable functional group, for example, an ethylenically unsaturated bond into the side chain of the polymer or introduction by formation of a salt structure between a polar substituent of the polymer resin and a compound containing a substituent having a counter charge to the polar substituent of the polymer resin and an ethylenically unsaturated bond is used.

Examples of the polymer having the ethylenically unsaturated bond in the side chain thereof include a polymer of an ester or amide of acrylic acid or methacrylic acid, wherein the ester or amide residue (R in  $-\text{COOR}$  or  $-\text{CONHR}$ ) has the ethylenically unsaturated bond. 25

Examples of the residue (R described above) having an ethylenically unsaturated bond include  $-(CH_2)_n$ ,  $CR_1=CR_2R_3$ ,  $-(CH_2O)_nCH_2CR_1=CR_2R_3$ ,  $-(CH_2CH_2O)_nCH_2CR_1=CR_2R_3$ ,  $-(CH_2)_nNH-CO-O-CH_2CR_1=CR_2R_3$ ,  $-(CH_2)_n-O-CO-CR_1=CR_2R_3$  and  $-(CH_2CH_2O)_2-X$  (wherein  $R_1$  to  $R_3$  each represents a hydrogen atom, a halogen atom or an alkyl group having from 1 to 20 carbon atoms, an aryl group, alkoxy group or aryloxy group, or  $R_1$  and  $R_2$  or  $R_1$  and  $R_3$  may be combined with each other to form a ring,  $n$  represents an integer of 1 to 10.  $X$  represents a dicyclopentadienyl residue). 40

Specific examples of the ester residue include  
 $-\text{CH}_2\text{CH}=\text{CH}_2$  (described in JP-B-7-21633)  
 $-\text{CH}_2\text{CH}_2\text{O}-\text{CH}_2\text{CH}=\text{CH}_2$ ,  $-\text{CH}_2\text{C}(\text{CH}_3)=\text{CH}_2$ ,  
 $-\text{CH}_2\text{CH}=\text{CH}-\text{C}_6\text{H}_5$ ,  $-\text{CH}_2\text{CH}_2\text{OCOCH}=\text{CH}-\text{C}_6\text{H}_5$ ,  
 $-\text{CH}_2\text{CH}_2\text{NHCOO}-\text{CH}_2\text{CH}=\text{CH}_2$  and  $-\text{CH}_2\text{CH}_2\text{O}-\text{X}$  45  
 (wherein X represents a dicyclopentadienyl residue).

Specific examples of the amide residue include  $-\text{CH}_2\text{CH}=\text{CH}_2$ ,  $-\text{CH}_2\text{CH}_2\text{O}-\text{Y}$  (wherein Y represents a cyclohexene residue) and  $-\text{CH}_2\text{CH}_2\text{OCO}-\text{CH}=\text{CH}_2$ .

As a monomer having a crosslinkable group for the polymer resin for undercoat layer, an ester or amide of acrylic acid or methacrylic acid having the crosslinkable group described above is preferably used.

The content of the crosslinkable group in the polymer resin for undercoat layer (content of the radical polymerizable unsaturated double bond determined by iodine titration) is preferably from 0.1 to 10.0 mmol, more preferably from 1.0 to 7.0 mmol, most preferably from 2.0 to 5.5 mmol, based on 1 g of the polymer resin. In the range described above, preferable compatibility between the sensitivity and stain resistance and good preservation stability can be achieved.

The weight average molecular weight (Mw) of the polymer resin for undercoat layer is preferably 5,000 or more, more preferably from 10,000 to 300,000. The number average molecular weight (Mn) of the polymer resin is preferably 1,000 or more, more preferably from 2,000 to 250,000. The polydispersity (Mw/Mn) thereof is preferably from 1.1 to 10.

The polymer resin for undercoat layer may be any of a random polymer, a block polymer, a graft polymer and the like, and is preferably a random polymer.

The polymer resins for undercoat layer may be used individually or in a mixture of two or more thereof.

The undercoat layer according to the invention may include a secondary amine or a tertiary amine. By the incorporation of the amino, the generation of spot-like stain is further prevented. Preferable examples of the secondary amine or tertiary amine include the following compounds.



In the invention, two or more kinds of the amines may be incorporated into the undercoat layer. The amount of the amine added to the undercoat layer is preferably from 10 to 90% by weight, more preferably from 20 to 80% by weight, most preferably from 30 to 70% by weight.

A coating solution for undercoat layer is obtained by dissolving the polymer resin for undercoat layer and other necessary component in an organic solvent (for example, methanol, ethanol, acetone or methyl ethyl ketone) and/or water. The coating solution for undercoat layer may contain an infrared absorbing agent.

In order to coat the coating solution for undercoat layer on the support, various known methods can be used. Examples of the method include bar coater coating, spin coating, spray coating, curtain coating, dip coating, air knife coating, blade coating and roll coating.

The coating amount (solid content) of the undercoat layer is preferably from 0.1 to 100 mg/m<sup>2</sup>, more preferably from 1 to 30 mg/m<sup>2</sup>.

[Lithographic Printing Method]

As the light source for use in the invention, a laser is preferable. The laser for use in the invention is not particularly restricted and preferably includes, for example, a solid laser or semiconductor laser emitting an infrared ray having a wavelength of 760 to 1,200 nm and a semiconductor laser emitting light having a wavelength of 250 to 420 nm.

With respect to the infrared ray laser, the output is preferably 100 mW or more, the exposure time per pixel is preferably within 20 microseconds, and the irradiation energy is preferably from 10 to 300 mJ/cm<sup>2</sup>. With respect to the semiconductor laser emitting light having a wavelength of 250 to 420 nm, the output is preferably 0.1 mW or more. In any of the laser exposures, it is preferred to use a multibeam laser device in order to shorten the exposure time.

The exposed lithographic printing plate precursor is mounted on a plate cylinder of a printing machine. In case of using a printing machine equipped with a laser exposure apparatus, the lithographic printing plate precursor is mounted on a plate cylinder of the printing machine and then subjected to the imagewise exposure.

After the imagewise exposure of the lithographic printing plate precursor by a laser, when dampening water and printing ink are supplied to perform printing without undergoing a development processing step, for example, a wet development processing step, in the exposed area of the image-recording layer, the image-recording layer cured by the exposure forms the printing ink receptive area having the oleophilic surface. On the other hand, in the unexposed area, the uncured image-recording layer is removed by dissolution or dispersion with the dampening water and/or printing ink supplied to reveal the hydrophilic surface in the area. As a result the dampening water adheres on the revealed hydrophilic surface and the printing ink adheres to the exposed area of the image-recording layer, whereby printing is initiated.

While either the dampening water or printing ink may be supplied at first on the surface of lithographic printing plate precursor, it is preferred to supply the printing ink at first in view of preventing the dampening water from contamination with the component of the image-recording layer removed. For the dampening water and printing ink, dampening water and printing ink for conventional lithographic printing are used respectively.

Thus, the lithographic printing plate precursor is subjected to the on-press development on an offset printing machine and used as it is for printing a large number of sheets.

## EXAMPLES

The present invention will be described in more detail with reference to the following examples, but the invention should not be construed as being limited thereto.

In the following examples, the effects of the compound according to the invention are examined with respect to lithographic printing plate precursors of types (I) to (III) having different image-recording layers and protective layers, respectively.

[I] Preparation of Lithographic Printing Plate Precursor of Type (I)

Example 1

(1) Preparation of Support

An aluminum plate (material: JIS A 1050) having a thickness of 0.3 mm was subjected to a degreasing treatment at 50° C. for 30 seconds using a 10% by weight aqueous sodium aluminate solution in order to remove rolling oil on the surface thereof and then grained the surface thereof using three nylon brushes embedded with bundles of nylon bristle having a diameter of 0.3 mm and an aqueous suspension (specific gravity: 1.1 g/cm<sup>3</sup>) of pumice having a median size of 25 µm, followed by thorough washing with water. The plate was subjected to etching by immersing in a 25% by weight aqueous sodium hydroxide solution of 45° C. for 9 seconds, washed with water, then immersed in a 20% by weight aqueous nitric acid solution at 60° C. for 20 seconds, and washed with water; The etching amount of the grained surface was about 3 g/m<sup>2</sup>.

Then, using an alternating current of 60 Hz, an electrochemical roughening treatment was continuously carried out on the plate. The electrolytic solution used was a 1% by weight aqueous nitric acid solution (containing 0.5% by weight of aluminum ion) and the temperature of electrolytic solution was 50° C. The electrochemical roughening treatment was conducted using an alternating current source, which provides a rectangular alternating current having a trapezoidal waveform such that the time TP necessary for the current value to reach the peak from zero was 0.8 msec and the duty ratio was 1:1, and using a carbon electrode as a counter electrode. A ferrite was used as an auxiliary anode. The current density was 30 A/dm<sup>2</sup> in terms of the peak value of the electric current, and 5% of the electric current flowing from the electric source was divided to the auxiliary anode. The quantity of electricity in the nitric acid electrolysis was 175 C/dm<sup>2</sup> in terms of the quantity of electricity when the aluminum plate functioned as an anode. The plate was then washed with water by spraying.

The plate was further subjected to an electrochemical roughening treatment in the same manner as in the nitric acid electrolysis above using as an electrolytic solution, a 0.5% by weight aqueous hydrochloric acid solution (containing 0.5% by weight of aluminum ion) having temperature of 50° C. and wider the condition that the quantity of electricity was 50 C/dm<sup>2</sup> in terms of the quantity of electricity when the aluminum plate functioned as an anode. The plate was then washed with water by spraying.

The plate was then subjected to an anodizing treatment using as an electrolytic solution, a 15% by weight aqueous sulfuric acid solution (containing 0.5% by weight of aluminum ion) at a current density of 15 A/dm<sup>2</sup> to form a direct current anodized film of 2.5 g/m<sup>2</sup>, washed with water and dried, thereby preparing Support (1).

Thereafter, in order to ensure the hydrophilicity of the non-image area, Support (1) was subjected to silicate treatment using an aqueous 1.5% by weight sodium silicate No. 3 solution at 70° C. for 12 seconds. The adhesion amount of Si was 6 mg/m<sup>2</sup>. Subsequently, the plate was washed with water to obtain Support (2). The center line average roughness (Ra) of Support (2) was measured using a stylus having a diameter of 2 µm and found to be 0.51 µm.

Undercoat solution (1) shown below was coated on Support (2) so as to have a dry coating amount of 20 mg/m<sup>2</sup> to prepare a support.

| <Undercoat solution (1)>                                                           |         |
|------------------------------------------------------------------------------------|---------|
| Undercoat compound (1) shown below                                                 | 0.18 g  |
| DABCO                                                                              | 0.12 g  |
| Methanol                                                                           | 55.24 g |
| Distilled water                                                                    | 6.15 g  |
|   |         |
|   |         |
|   |         |
|   |         |
|  |         |
|  |         |
| (Mw: 80,000)                                                                       |         |
| Undercoat compound (1)                                                             |         |

## (2) Formation of Image-Recording Layer

Coating solution (1) for image-recording layer having the composition shown below was coated on the support provided with the undercoat layer by a bar and dried in an oven at 100° C. for 60 seconds to form an image-recording layer having a dry coating amount of 1.0 g/m<sup>2</sup>.

Coating solution (1) for image-recording layer was prepared by mixing Photosensitive solution (1) shown below with Microgel solution (1) shown below just before the coating, followed by stirring.

| <Photosensitive solution (1)>                                                                                                                |         |
|----------------------------------------------------------------------------------------------------------------------------------------------|---------|
| Binder polymer (1) having structure shown below                                                                                              | 0.240 g |
| Infrared absorbing agent (1) having structure shown below [Component (A)]                                                                    | 0.030 g |
| Polymerization initiator (1) having structure shown below [Component (B)]                                                                    | 0.162 g |
| Polymerizable compound (tris(acryloyloxyethyl) isocyanurate (NK Ester A-9300, produced by Shin-Nakamura Chemical Co., Ltd.)) [Component (C)] | 0.192 g |
| Tris(2-hydroxyethyl) isocyanurate                                                                                                            | 0.062 g |
| Benzyl dimethyl octyl ammonium PF <sub>6</sub> <sup>-</sup> salt                                                                             | 0.018 g |
| Compound A-(1) according to invention (W-BJ, produced by Fuji Film Co., Ltd.)                                                                | 0.055 g |
| Fluorine-based surfactant (1) having structure shown below                                                                                   | 0.008 g |
| Methyl ethyl ketone                                                                                                                          | 1.091 g |
| 1-Methoxy-2-propanol                                                                                                                         | 8.609 g |

| <Microgel solution (1)> |                                                                                      |
|-------------------------|--------------------------------------------------------------------------------------|
| 5                       | Microgel (1) shown below                                                             |
|                         | Distilled water                                                                      |
| 5                       | 2.640 g                                                                              |
|                         | 2.425 g                                                                              |
| 10                      |     |
| 10                      |    |
| 15                      |    |
| 20                      | (Mw: 70,000)<br>Binder polymer (1)                                                   |
| 25                      |   |
| 30                      | Infrared absorbing agent (1)                                                         |
| 35                      |  |
| 35                      | Polymerization initiator (1)                                                         |
| 40                      |  |
| 45                      | Fluorine-based surfactant (1)                                                        |
| 50                      | (Mw: 13,000)                                                                         |

## (Preparation of Microgel (1))

An oil phase component was prepared by dissolving 10 g of adduct of trimethylol propane and xylene diisocyanate (Takeneate D-110N, produced by Mitsui Takeda Chemical Co., Ltd.), 3.15 g of pentaerythritol triacetate (SR444, produced by Nippon Kayaku Co., Ltd.) and 0.1 g of Pionine A-41C (produced by Takemoto Oil and Fat Co., Ltd.) in 17 g of ethyl acetate. As an aqueous phase component, 40 g of a 4% by weight aqueous solution of PVA-205 was prepared. The oil phase component and the aqueous phase component were mixed and emulsified using a homogenizer at 12,000 rpm for 10 minutes. The resulting emulsion was added to 25 g of distilled water and stirred at room temperature for 30 minutes

and then at 50° C. for 3 hours. The microgel liquid thus-obtained was diluted using distilled water so as to have the solid concentration of 15% by weight to prepare Microgel (1). The average particle size of Microgel (1) was 0.2  $\mu$ m.

### (3) Formation of Protective Layer

Coating solution (1) for protective layer having the composition shown below was coated on the image-recording layer described above by a bar and dried in an oven at 120° C. for 60 seconds to form a protective layer having a dry coating amount of 0.15 g/m<sup>2</sup>, thereby preparing a lithographic printing plate precursor of Example 1.

| <Coating solution (1) for protective layer>                                                                                                                                                                           |        |
|-----------------------------------------------------------------------------------------------------------------------------------------------------------------------------------------------------------------------|--------|
| Dispersion of inorganic stratiform compound (1) shown below                                                                                                                                                           | 1.5 g  |
| Aqueous 6% by weight solution of polyvinyl alcohol (CKS 50, sulfonic acid-modified, saponification degree: 99% by mole or more, polymerization degree: 300, produced by Nippon Synthetic Chemical Industry Co., Ltd.) | 0.55 g |
| Aqueous 6% by weight solution of polyvinyl alcohol (PVA-405, saponification degree: 81.5% by mole, polymerization degree: 500, produced by Kuraray Co., Ltd.)                                                         | 0.03 g |
| Aqueous 1% by weight solution of surfactant (Emalex 710, produced by Nihon Emulsion Co., Ltd.)                                                                                                                        | 8.60 g |
| Ion-exchanged water                                                                                                                                                                                                   | 6.0 g  |

## (Preparation of Dispersion of Inorganic Stratiform Compound (1))

To 193.6 g of ion-exchanged water was added 6.4 g of synthetic mica (Somasif M-100, produced by CO-OP Chemical Co., Ltd.) and the mixture was dispersed using a homogenizer until an average particle size (according to a laser scattering method) became 3  $\mu\text{m}$  to prepare Dispersion of inorganic stratiform compound (1). The aspect ratio of the inorganic particle thus-dispersed was 100 or more.

## Examples 2 to 14 and 17 to 27 and Comparative Examples 1 to 5

Lithographic printing plate precursors of Examples 2 to 14 and 17 to 27 and Comparative Examples 1 to 5 were prepared in the same manner as in Example 1 except for changing Compound A-(1) according to the invention contained in Photosensitive solution (1) for the lithographic printing plate precursor of Example 1 to the compounds shown in Table 1, respectively. Compound B-(1) according to the invention is Beaulight ESS produced by Sanyo Chemical Industries, Ltd.

### Example 15

A lithographic printing plate precursor was prepared in the same manner as in Example 1 except for changing Undercoat solution (1) used in Example 1 to Undercoat solution (2) shown below.

| <Undercoat solution (2)>              |         |
|---------------------------------------|---------|
| Undercoat compound (1) shown above    | 0.18 g  |
| DABCO                                 | 0.12 g  |
| Compound A-(1) according to invention | 0.15 g  |
| Methanol                              | 55.24 g |
| Distilled water                       | 6.15 g  |

### Example 16

A lithographic printing plate precursor was prepared in the same manner as in Example 15 except for using a photo-

sitive solution prepared by eliminating Compound A-(1) according to invention from Photosensitive solution (1) used in example 15.

### Example 28

A lithographic printing plate precursor was prepared in the same manner as in Example 17 except for changing Undercoat solution (1) used in Example 17 to Undercoat solution (3) shown below.

| <Undercoat solution (3)> |                                              |
|--------------------------|----------------------------------------------|
| 15                       | Undercoat compound (1) shown above 0.18 g    |
|                          | DABCO 0.12 g                                 |
|                          | Compound B-(1) according to invention 0.15 g |
|                          | Methanol 55.24 g                             |
|                          | Distilled water 6.15 g                       |

### Example 29

A lithographic printing plate precursor was prepared in the same manner as in Example 28 except for using a photosensitive solution prepared by eliminating Compound B-(1) according to invention from Photosensitive solution (1) used in example 28.

[II] Preparation of Lithographic Printing Plate Precursor of  
30 Type (II)

### Example 30

A lithographic printing plate precursor of Example 30 was prepared in the same manner as in Example 1 except for changing Coating solution (1) for image-recording layer used in Example 1 to Coating solution (2) for image-recording layer shown below.

| <Coating solution (2) for image-recording layer> |                                                                                          |
|--------------------------------------------------|------------------------------------------------------------------------------------------|
| 40                                               | Binder polymer (1) shown above 0.50 g                                                    |
|                                                  | Infrared absorbing agent (2) shown below 0.05 g                                          |
| 45                                               | Polymerization initiator (1) shown above 0.20 g                                          |
|                                                  | Polymerizable compound (Aronics M-215, produced by 1.00 g<br>Toagosei Co., Ltd.)         |
|                                                  | Compound A-(1) according to invention (W-BJ1, produced by 0.05 g<br>Fuji Film Co., Ltd.) |
|                                                  | Fluorine-based surfactant (1) shown above 0.10 g                                         |
| 50                                               | Methyl ethyl ketone 18.0 g                                                               |



## Examples 31 to 39 and Comparative Examples 6 to 10

65 Lithographic printing plate precursors of Examples 31 to 39 and Comparative Examples 6 to 10 were prepared in the same manner as in Example 30 except for changing Com-

pound A-(1) according to the invention contained in Coating solution (2) for image-recording layer to the compounds shown in Table 2, respectively.

[III] Preparation of Lithographic Printing Plate Precursor of Type (III)

#### Example 40

Coating solution (3) for image-recording layer shown below was coated on the same support provided with the undercoat layer as described in Example 1 by a bar and dried in an oven at 70° C. for 60 seconds to form an image-recording layer having a dry coating amount of 0.6 g/m<sup>2</sup>.

| <Coating solution (3) for image-recording layer>                                     |        |
|--------------------------------------------------------------------------------------|--------|
| Aqueous dispersion of polymer fine particle (hydrophobilizing precursor) shown below | 33.0 g |
| Infrared absorbing agent (3) shown below                                             | 1.0 g  |
| Pentaerythritol tetraacrylate                                                        | 0.5 g  |
| Compound A-(1) according to invention (W-BJ, produced by Fuji Film Co., Ltd.)        | 0.1 g  |
| Methanol                                                                             | 16.0 g |



#### (Preparation of Aqueous Dispersion of Polymer Fine Particle (Hydrophobilizing Precursor))

A stirrer, a thermometer, a dropping funnel, a nitrogen inlet tube and a reflux condenser were attached to a 1,000 ml four-neck flask and while carrying out deoxygenation by introduction of nitrogen gas, 350 ml of distilled water was charged therein and heated until the internal temperature reached 80° C. To the flask was added 3.0 g of sodium dodecylsulfate as a dispersing agent, then was added 0.45 g of ammonium persulfate as an initiator, and thereafter was dropwise added a mixture of 45.0 g of glycidyl methacrylate and 45.0 g of styrene through the dropping funnel over a period of about one hour. After the completion of the dropwise addition, the mixture was continued to react as it was for 5 hours, followed by removing the unreacted monomers by steam distillation. The mixture was cooled, adjusted the pH to 6 with aqueous ammonia and finally added pure water thereto so as to have the nonvolatile content of 15% by weight to obtain an aqueous dispersion of polymer fine particle (hydrophobilizing precursor). The particle size distribution of the polymer fine particle had the maximum value at the particle size of 60 nm.

The particle size distribution was determined by taking an electron micrograph of the polymer fine particle, measuring particle sizes of 5,000 fine particles in total on the photograph, and dividing a range from the largest value of the particle size measured to 0 on a logarithmic scale into 50 parts to obtain occurrence frequency of each particle size by plotting. With respect to the aspherical particle, a particle size of a spherical particle having a particle area equivalent to the particle area of the aspherical particle on the photograph was defined as the particle size.

Coating solution (2) for protective layer shown below was coated on the image-recording layer thus-prepared by a bar

and dried in an oven at 60° C. for 120 seconds to form a protective layer having a dry coating amount of 0.3 μm<sup>2</sup>, thereby preparing a lithographic printing plate precursor of Example 40.

5

| <Coating solution (2) for protective layer> |        |  |
|---------------------------------------------|--------|--|
| Carboxymethyl cellulose (Mw: 20,000)        | 5.0 g  |  |
| Water                                       | 50.0 g |  |

#### Examples 41 to 49 and Comparative Examples 10 to 15

15

Lithographic printing plate precursors of Examples 41 to 49 and Comparative Examples 11 to 15 were prepared in the same manner as in Example 40 except for changing Compound A-(1) according to the invention contained in Coating solution (3) for image-recording layer to the compounds shown in Table 3, respectively.

#### [Evaluation of Lithographic Printing Plate Precursor]

Each of the lithographic printing plate precursors thus-obtained was exposed by Luxel Platesetter T-6000III equipped with an infrared semiconductor laser, produced by Fuji Film Co., Ltd. under the conditions of a rotational number of outer surface drum of 1,000 rpm, a laser output of 70% and a resolution of 2,400 dpi. The exposed image contained a solid image and a 50% halftone dot chart of a 20 μm-dot FM screen.

The exposed lithographic printing plate precursor was mounted without conducting development processing on a plate cylinder of a printing machine (Lithrone 26, produced by Komori Corp.). Using dampening water (Ecolity-2 (produced by Fuji Film Co., Ltd.)/tap water=2/98 (volume ratio)) and Values-G A Black Ink (produced by Dainippon Ink & Chemicals, Inc.), the dampening water and ink were supplied according to the standard automatic printing start method of Lithrone 26 to conduct printing on 100 sheets of Tokubishi art paper (76.5 kg) at a printing speed of 10,000 sheets per hour.

#### (A) On-Press Development Property

A number of the printing papers required until the on-press development of the unexposed area of the image-recording layer on the printing machine was completed to reach a state where the ink was not transferred to the printing paper in the non-image area was measured to evaluate the on-press development property. The results obtained are shown in Tables 1 to 3.

#### (B) Spot-Like Printing Stain

Each of the lithographic printing plate precursors was allowed to stand in a constant temperature and humidity chamber set at temperature of 45° C. and relative humidity of 75% for 3 days. Then, the lithographic printing plate precursor was mounted without image exposure on the printing machine and subjected to the on-press development by supplying the dampening water and ink in the same manner as described above. At the completion of the on-press development, the number of fine spot-like stains generated in 100 cm<sup>2</sup> area of the printing paper was counted. The results obtained are shown in Tables 1 to 3.

In Tables 1 to 3, the compounds according to the invention are indicated using the numbers of the compounds illustrated hereinbefore. The compounds for comparison used are shown below.

## Compounds for Comparison

TABLE 1

| Lithographic Printing Plate Precursor of Type (I) |                                                            |                                                  |                                                        |
|---------------------------------------------------|------------------------------------------------------------|--------------------------------------------------|--------------------------------------------------------|
|                                                   | Compound according to Invention or Compound for Comparison | On-press Development Property (number of sheets) | Spot-like Printing Stain (number/100 cm <sup>2</sup> ) |
| Example 1                                         | A-(1)                                                      | 20                                               | 30                                                     |
| Example 2                                         | A-(2)                                                      | 20                                               | 35                                                     |
| Example 3                                         | A-(4)                                                      | 10                                               | 5                                                      |
| Example 4                                         | A-(6)                                                      | 15                                               | 10                                                     |
| Example 5                                         | A-(7)                                                      | 20                                               | 25                                                     |
| Example 6                                         | A-(8)                                                      | 15                                               | 10                                                     |
| Example 7                                         | A-(10)                                                     | 20                                               | 20                                                     |
| Example 8                                         | A-(11)                                                     | 15                                               | 5                                                      |
| Example 9                                         | A-(14)                                                     | 20                                               | 10                                                     |
| Example 10                                        | A-(20)                                                     | 15                                               | 20                                                     |
| Example 11                                        | A-(25)                                                     | 10                                               | 5                                                      |
| Example 12                                        | A-(29)                                                     | 10                                               | 5                                                      |
| Example 13                                        | A-(34)                                                     | 5                                                | 5                                                      |
| Example 14                                        | A-(35)                                                     | 5                                                | 5                                                      |
| Example 15                                        | A-(1)                                                      | 10                                               | 20                                                     |
| Example 16                                        | A-(1)                                                      | 20                                               | 30                                                     |
| Comparative                                       | (I)                                                        | 25                                               | 135                                                    |
| Example 1                                         |                                                            |                                                  |                                                        |
| Comparative                                       | (III)                                                      | 45                                               | 120                                                    |
| Example 2                                         |                                                            |                                                  |                                                        |
| Comparative                                       | (IV)                                                       | 30                                               | 130                                                    |
| Example 3                                         |                                                            |                                                  |                                                        |
| Comparative                                       | (V)                                                        | 70                                               | 70                                                     |
| Example 4                                         |                                                            |                                                  |                                                        |
| Comparative                                       | (VI)                                                       | 55                                               | 110                                                    |
| Example 5                                         |                                                            |                                                  |                                                        |
| Example 17                                        | B-(1)                                                      | 10                                               | 20                                                     |
| Example 18                                        | B-(2)                                                      | 5                                                | 15                                                     |
| Example 19                                        | B-(2)(0.011 g) + B-(2')(0.044 g)                           | 5                                                | 5                                                      |
| Example 20                                        | B-(5)                                                      | 5                                                | 10                                                     |
| Example 21                                        | B-(6)                                                      | 5                                                | 10                                                     |
| Example 22                                        | B-(8)                                                      | 15                                               | 30                                                     |
| Example 23                                        | B-(13)                                                     | 5                                                | 5                                                      |
| Example 24                                        | B-(14)                                                     | 5                                                | 5                                                      |
| Example 25                                        | B-(15)                                                     | 5                                                | 25                                                     |
| Example 26                                        | B-(16)                                                     | 5                                                | 15                                                     |
| Example 27                                        | B-(17)                                                     | 5                                                | 10                                                     |
| Example 28                                        | B-(1)                                                      | 5                                                | 10                                                     |
| Example 29                                        | B-(1)                                                      | 10                                               | 20                                                     |



TABLE 1-continued



TABLE 2

| Lithographic Printing Plate Precursor of Type (II) |                                                            |                                                  |                                                        |
|----------------------------------------------------|------------------------------------------------------------|--------------------------------------------------|--------------------------------------------------------|
|                                                    | Compound according to Invention or Compound for Comparison | On-press Development Property (number of sheets) | Spot-like Printing Stain (number/100 cm <sup>2</sup> ) |
| Example 30                                         | A-(1)                                                      | 25                                               | 15                                                     |
| Example 31                                         | A-(4)                                                      | 15                                               | 5                                                      |
| Example 32                                         | A-(7)                                                      | 25                                               | 10                                                     |
| Example 33                                         | A-(13)                                                     | 20                                               | 5                                                      |
| Example 34                                         | A-(20)                                                     | 25                                               | 20                                                     |
| Comparative                                        | (I)                                                        | 35                                               | 110                                                    |
| Example 6                                          | Comparative (III)                                          | 55                                               | 100                                                    |
| Example 7                                          | Comparative (IV)                                           | 40                                               | 110                                                    |
| Example 8                                          | Comparative (V)                                            | 85                                               | 55                                                     |
| Example 9                                          | Comparative (VI)                                           | 70                                               | 85                                                     |
| Example 10                                         |                                                            |                                                  |                                                        |
| Example 35                                         | B-(1)                                                      | 15                                               | 30                                                     |
| Example 36                                         | B-(2)                                                      | 10                                               | 20                                                     |
| Example 37                                         | B-(6)                                                      | 10                                               | 20                                                     |
| Example 38                                         | B-(14)                                                     | 5                                                | 10                                                     |
| Example 39                                         | B-(17)                                                     | 5                                                | 15                                                     |

TABLE 3

| Lithographic Printing Plate Precursor of Type (III) |                                                            |                                                  |                                                        |
|-----------------------------------------------------|------------------------------------------------------------|--------------------------------------------------|--------------------------------------------------------|
|                                                     | Compound according to Invention or Compound for Comparison | On-press Development Property (number of sheets) | Spot-like Printing Stain (number/100 cm <sup>2</sup> ) |
| Example 40                                          | A-(1)                                                      | 25                                               | 15                                                     |
| Example 41                                          | A-(6)                                                      | 15                                               | 5                                                      |
| Example 42                                          | A-(9)                                                      | 25                                               | 15                                                     |
| Example 43                                          | A-(11)                                                     | 25                                               | 5                                                      |
| Example 44                                          | A-(20)                                                     | 30                                               | 20                                                     |
| Comparative                                         | (I)                                                        | 50                                               | 105                                                    |
| Example 11                                          | Comparative (III)                                          | 70                                               | 90                                                     |
| Example 12                                          | Comparative (IV)                                           | 60                                               | 100                                                    |
| Example 13                                          | Comparative (V)                                            | 110                                              | 45                                                     |
| Example 14                                          | Comparative (VI)                                           | 90                                               | 70                                                     |
| Example 15                                          |                                                            |                                                  |                                                        |
| Example 45                                          | B-(1)                                                      | 15                                               | 30                                                     |
| Example 46                                          | B-(2)                                                      | 10                                               | 25                                                     |
| Example 47                                          | B-(6)                                                      | 15                                               | 20                                                     |
| Example 48                                          | B-(13)                                                     | 10                                               | 10                                                     |
| Example 49                                          | B-(18)                                                     | 10                                               | 10                                                     |

As is apparent from the results shown in Tables 1 to 3, the good compatibility of good on-press development property and prevention of spot-like printing stain can be achieved according to the lithographic printing plate precursor of the invention.

What is claimed is:

1. A lithographic printing plate precursor capable of being subjected to on-press development by supplying at least one of printing ink and dampening water and comprising a support, an image-recording layer and optionally an undercoat layer between the support and the image-recording layer, wherein at least one of the undercoat layer and the image-recording layer comprises at least one of

a compound represented by the following formula (IA),



wherein, R represents a substituted or unsubstituted alkyl group, Z represents a polyoxyethylene group or a polyoxypropylene group, Y represents a substituted or unsubstituted alkylene group having 18 or less carbon atoms, a substituted or unsubstituted arylene group having 30 or less carbon atoms or a divalent heterocyclic group, and X represents a sulfonate.

2. The lithographic printing plate precursor as claimed in claim 1, wherein the image-recording layer comprises an infrared absorbing agent, a polymerization initiator and a polymerizable compound.

3. The lithographic printing plate precursor as claimed in claim 1, which further comprises a protective layer so that the support, the image-recording layer and the protective layer are provided in this order.

4. The lithographic printing plate precursor as claimed in claim 1, wherein Y of formula (IA) is a substituted or unsubstituted butylene group.

5. The lithographic printing plate precursor as claimed in claim 4, wherein R of formula (IA) is a branched alkyl group having from 1 to 30 carbon atoms.

6. The lithographic printing plate precursor as claimed in claim 4, wherein Z in the formula (IA) is a polyoxyethylene group having a repeating unit number of from 3 to 40 or a polyoxypropylene group having a repeating unit number of from 3 to 40.

7. The lithographic printing plate precursor as claimed in claim 1, wherein R of formula (IA) is a branched alkyl group having from 1 to 30 carbon atoms.

8. A lithographic printing plate precursor capable of being subjected to on-press development by supplying at least one of printing ink and dampening water and comprising a support, an image-recording layer and optionally an undercoat layer between the support and the image-recording layer, wherein at least one of the undercoat layer and the image-recording layer comprises at least one of

a compound represented by the following formula (IA),



wherein

R represents a substituted or unsubstituted alkyl group Z in the formula (IA) is a polyoxyethylene group having a repeating unit number of from 3 to 40 or a polyoxypropylene group having a repeating unit number of from 3 to 40, Y represents a substituted or unsubstituted alkylene group having 18 or less carbon atoms, a substituted or unsubstituted arylene group having 30 or less carbon atoms or a divalent heterocyclic group and X represents a sulfonate.

\* \* \* \* \*